# EUROPEAN PATENT SPECIFICATION

(11) **EP 4 172 395 B1**
(45) Date of publication and mention of the grant of the patent: **05.08.2026**
(21) Application number: 21739838.7
(22) Date of filing: 14.06.2021
(51) Int. Cl.: D04H 1/425, D04H 1/541, A41D 31/06, B68G 1/00

(54) **WASHABLE CELLULOSE ACETATE FIBER BLENDS FOR THERMAL INSULATION**
WASCHBARE CELLULOSEACETATFASERMISCHUNGEN ZUR WÄRMEDÄMMUNG
MÉLANGES DE FIBRES LAVABLES D'ACÉTATE DE CELLULOSE POUR ISOLATION THERMIQUE

(30) Priority: 30.06.2020 US 202063046283 P
(43) Date of publication of application: 03.05.2023
(73) Proprietor: Eastman Chemical Company, Kingsport, TN 37660 (US)
(72) Inventor: EDWARDS, Brian Tyndall, Jonesborough, TN 37659 (US); SATAM, Dnyanada Shankar, Boca Raton, FL 33428 (US); HELTON, Megan Danielle, Kingsport, TN 37663 (US); BARHAM, Kevin Todd, Kingsport, TN 37663 (US); ROGERS-SMITH, Ariana Maurique, Kingsport, TN 37664 (US)
(74) Representative: Ricker, Mathias
(86) International application number: PCT/US2021/037183
(87) International publication number: WO 2022/005729

(56) References cited:
- WO-A1-2014/116439
- WO-A1-2018/160584
- WO-A1-2020/046634
- CA-A- 677 852
- US-A- 4 129 675

## Description

### FIELD OF THE INVENTION

The invention generally relates to fiber blends useful as a thermal insulation batting. It particularly relates to blends containing sustainably derived cellulose acetate fibers, which can be made into loose fill fibers or nonwoven webs for heat-bonding or resin bonding and subsequent use as thermal insulation, for example, in garments and bedding, and have good loft and thermal insulation after multiple wash cycles.

### BACKGROUND OF THE INVENTION

One of nature's best thermal insulators is down. Down insulation is typically made from goose or duck plumage-the lofty, fluffy layer underneath the feathers. Down creates high-loft clusters that trap air and body heat. In addition to its ability to efficiently trap heat, down is compressible and provides excellent thermal resistance properties at low weights.

Down insulation, however, has several drawbacks including losing its loft as well as its insulating power when wet making it a poor choice for environments that are both cold and wet. Down insulation is also relatively expensive and poses animal welfare concerns.

A typical alternative to down insulation is a polyester nonwoven insulation batting. The batting can include short-staple or continuous polyester filament. While it addresses some of the concerns of down in terms of loft retention while wet and animal welfare, it is sourced from petroleum, and the fiber is essentially non-biodegradable and non-compostable.

The fiber selected desirably should have a good compression recovery. Fiber batting is typically shipped in a compressed state to reduce shipping costs. Upon releasing the bale from its compressed state, the fiber batting desirably recovers as much of its original loft as possible. Many fibers, while having a suitable initial loft, do not recover well after undergoing a state of compression.

Thus, there is a need in the art to provide the industry with fibers that can be used with and/or polyester fibers that provide acceptable insulation power and loft retention after washing cycles, can recover at least more than half of its loft after compression, and also be derived from sustainable resources. Optionally, such fibers are biodegradable.

Cellulose acetate fiber blends for thermal insulation batting are disclosed in WO 2020/046634.

The present invention addresses this need as well as others, which will become apparent from the following description and the appended claims.

### SUMMARY OF THE INVENTION

The invention is as set forth in the appended claims.

There is now provided a staple fiber blend comprising:
(a) a cellulose acetate staple fibers having a denier per filament (dpf) of 3.0 or less, in an amount ranging from 45 to 60 wt% based on the total weight of the fiber blend; and
(b) structural staple fibers having a dpf of 6.0 or more, in an amount ranging from 20 to 35 wt% based on the total weight of the fiber blend; and
(c) binder fibers, in an amount ranging from 0 to 30 wt % based on the total weight of the fiber blend.

The structural fibers can be cellulose acetate fibers, polyester fibers, or other types of structural fibers such as acrylics.

There is also provided a nonwoven web comprising this fiber blend, as well as battings, fiber fill, interliners, and even bales with the fiber blend.

Articles such as garments, shoes, gloves, pillows, comforters, blankets, throw blankets, mattresses, mattress pads, sleeping bags, and cushions can be made with these fiber blends.

### BRIEF DESCRIPTION OF THE DRAWINGS

Figure 1 is a diagram showing the preparation of the samples used for testing in the wash cycles.
Figure 2 is a graph illustrating the thermal insulation trends after multiple wash cycles of non-woven webs made with CA fibers relative to other commercial products.
Figure 3 is a graph illustrating the thermal insulation per unit basis weight after multiple wash cycles of non-woven webs made with CA fibers relative to other commercial products.
Figure 4 is a graph illustrating the loft trends after multiple wash cycles of non-woven webs made with CA fibers relative to other commercial products.
Figure 5 is a bar chart illustrating the compression resistance of the non-woven webs made with varying amounts and dpf types of CA fibers.
Figure 6 is a bar chart illustrating the short term compression recovery of the non-woven webs made with varying amounts and dpf types of CA fibers.

### DETAILED DESCRIPTION OF THE INVENTION

It has been discovered that a fiber blend and nonwoven webs derived from the fiber blend can provide loft retention and insulation values (clo) after several wash cycles that are comparable to all polyester or polyester/nylon blends, yet contain fibers that are sustainably derived, and optionally can be biodegradable. We have also found that the particular attribute desired in the application containing the fiber blend can be emphasized by dialing in the amount and morphology of the cellulose acetate fiber. In some cases, it is now possible to obtain a fiber batting that has a significant loft recovery after compression, and in some cases, a higher loft recovery that battings made with 100% of the higher dpf structural fibers.

The fiber blend contains a staple cellulose acetate fiber having a denier per filament (dpf) of 3.0 or less. The CA fibers having a dpf of not more than 3.0 provide a soft hand feel and increase the battings ability to trap pockets of still air, thereby provided a batting, non-woven web, interliners, and articles having a good clo insulation values as well as an initial loft. A staple fiber "blend" includes loose fiber fills, non-woven webs, interliners, battings, and the fiber content of any of the articles described herein.

Useful cellulose acetate (CA) staple fibers are described in Int'l Patent Application No. WO 2018/160584 filed on February 27, 2018.

The CA fibers are sustainable because they are derived from a cellulosic backbone obtained from plants such as wood or cotton.

As used herein, a cellulose acetate fibers or CA fibers includes cellulose diacetate, cellulose triacetate, cellulose acetate propionate, and cellulose acetate butyrate, or mixtures thereof. CA fibers as used herein are distinct from and do not include within its class the regenerated cellulose typically under the generic name of rayon such as viscose, modal, and lyocell including Tencell and Lycra. The CA can have a degree of substitution ranging from 1.9 to less than 3. As used herein, the term "degree of substitution" or "DS" refers to the average number of acyl substituents per anhydroglucose ring of the cellulose polymer, wherein the maximum degree of substitution is 3.0. In some cases, the CA may have an average degree of substitution of at least 1.95, 2.0, 2.05, 2.1, 2.15, 2.2, 2.25, or 2.3 and/or not more than 2.9, 2.85, 2.8, 2.75, 2.7, 2.65, 2.6, 2.55, 2.5, 2.45, 2.4, or 2.35. The DS may also fall within one or more of the above ranges (e.g., from 2.2 to 2.8). In some cases, at least 90, 91, 92, 93, 94, 95, 96, 97, 98, or 99 percent of the CA has a DS of greater than 2.15, 2.2, or 2.25. In some cases, at least 90 percent of the CA can have a DS of greater than 2.2, 2.25, 2.3, or 2.35. Typically, acetyl groups can make up at least 1, 5, 10, 15, 20, 25, 30, 35, 40, 45, 50, 55, or 60 percent and/or not more than 99, 95, 90, 85, 80, 75, or 70 percent of the total acyl substituents.

The CA fibers may have a weight-average molecular weight (M_{w}) of not more than 90,000, measured using gel permeation chromatography with N-methyl-2-pyrrolidone (NMP) as the solvent. In some case, the CA may have a M_{w} of at least 10,000, at least 20,000, 25,000, 30,000, 35,000, 40,000, or 45,000 and/or not more than 100,000, 95,000, 90,000, 85,000, 80,000, 75,000, 70,000, 65,000, 60,000, or 50,000.

The CA fibers may be formed by any suitable method. In some cases, the CA may be formed by reacting a cellulosic material such as wood pulp with acetic anhydride and a catalyst in an acidic reaction medium to form a CA flake. The flake may then be dissolved in a solvent, such as acetone or methyl ethyl ketone, to form a "solvent dope," which can be filtered and sent through a spinnerette to form CA fibers. In some cases, up to 1 weight percent or more of titanium dioxide or other delusterant may be added to the dope prior to filtration, depending on the desired properties and ultimate end-use of the fibers.

In some cases, the solvent dope or flake used to form the CA fibers may include few or no additives in addition to the CE. Such additives can include, but are not limited to, plasticizers, antioxidants, thermal stabilizers, pro-oxidants, acid scavengers, inorganics, pigments, and colorants. In some cases, the CA fibers can include at least 90, 90.5, 91, 91.5, 92, 92.5, 93, 93.5, 94, 94.5, 95, 95.5, 96, 96.5, 97, 97.5, 98, 98.5, 99, 99.5, 99.9, 99.99, 99.995, or 99.999 percent of CE, based on the total weight of the fiber. The CA fibers may include not more than 10, 9.5, 9, 8.5, 8, 7.5, 7, 6.5, 6, 5.5, 5, 4.5, 4, 3.5, 3, 2.5, 2, 1.5, 1, 0.5, 0.1, 0.01, 0.005, or 0.001 weight percent of additives, including the specific additives listed herein.

The CA fibers can achieve higher levels of biodegradability and/or compostability without using additives that have traditionally been used to facilitate environmental non-persistence of similar fibers. Such additives can include, for example, photodegradation agents, biodegradation agents, decomposition accelerating agents, and various types of other additives. In some cases, despite being substantially free of these types of additives, the CA fibers and articles can exhibit enhanced biodegradability and compostability when tested under industrial, home, and/or soil conditions.

In some embodiments, the CA fibers may be substantially free of photodegradation agents. For example, the fibers may include not more than 1, 0.75, 0.50, 0.25, 0.10, 0.05, 0.025, 0.01, 0.005, 0.0025, or 0.001 weight percent of photodegradation agent, based on the total weight of the fiber, or the fibers may include no photodegradation agents. Examples of such photodegradation agents include, but are not limited to, pigments which act as photooxidation catalysts and are optionally augmented by the presence of one or more metal salts, oxidizable promoters, and combinations thereof. Pigments can include coated or uncoated anatase or rutile titanium dioxide, which may be present alone or in combination with one or more of the augmenting components such as, for example, various types of metals. Other examples of photodegradation agents include benzoins, benzoin alkyl ethers, benzophenone and its derivatives, acetophenone and its derivatives, quinones, thioxanthones, phthalocyanine and other photosensitizers, ethylene-carbon monoxide copolymer, aromatic ketone-metal salt sensitizers, and combinations thereof.

In some embodiments, the CA fibers may be substantially free of biodegradation agents and/or decomposition agents. For example, the fibers may include not more than 1, 0.75, 0.50, 0.25, 0.10, 0.05, 0.025, 0.01, 0.005, 0.0025, 0.0020, 0.0015, 0.001, 0.0005 weight percent of biodegradation agents and/or decomposition agents, based on the total weight of the fiber, or the fibers may include no biodegradation and/or decomposition agents. Examples of such biodegradation and decomposition agents include, but are not limited to, salts of oxygen acid of phosphorus, esters of oxygen acid of phosphorus or salts thereof, carbonic acids or salts thereof, oxygen acids of phosphorus, oxygen acids of sulfur, oxygen acids of nitrogen, partial esters or hydrogen salts of these oxygen acids, carbonic acid and its hydrogen salt, sulfonic acids, and carboxylic acids.

Other examples of such biodegradation and decomposition agents include an organic acid selected from the group consisting of oxo acids having 2 to 6 carbon atoms per molecule, saturated dicarboxylic acids having 2 to 6 carbon atoms per molecule, and lower alkyl esters of the oxo acids or the saturated dicarboxylic acids with alcohols having from 1 to 4 carbon atoms. Biodegradation agents may also comprise enzymes such as, for example, a lipase, a cellulase, an esterase, and combinations thereof. Other types of biodegradation and decomposition agents can include cellulose phosphate, starch phosphate, calcium secondary phosphate, calcium tertiary phosphate, calcium phosphate hydroxide, glycolic acid, lactic acid, citric acid, tartaric acid, malic acid, oxalic acid, malonic acid, succinic acid, succinic anhydride, glutaric acid, acetic acid, and combinations thereof.

The CA fibers may also be substantially free of several other types of additives that have been added to other fibers to encourage environmental non-persistence. Examples of these additives can include, but are not limited to, polyesters, including aliphatic and low molecular weight (e.g., less than 5000) polyesters, enzymes, microorganisms, water soluble polymers, modified cellulose acetate, water-dispersible additives, nitrogen-containing compounds, hydroxy-functional compounds, oxygen-containing heterocyclic compounds, sulfur-containing heterocyclic compounds, anhydrides, monoepoxides, and combinations thereof. In some cases, the CA fibers may include not more than 0.5, 0.4, 0.3, 0.25, 0.1, 0.075, 0.05, 0.025, 0.01, 0.0075, 0.005, 0.0025, or 0.001 weight percent of these types of additives, or the CA fibers may not include any of these types of additives.

At the spinnerette, the solvent dope can be extruded through a plurality of holes to form continuous cellulose acetate filaments. The filaments may be gathered together to form bundles of several hundred, or even thousand, individual filaments. Each of these bundles, or bands, may include at least 100, 150, 200, 250, 300, 350, or 400 and/or not more than 1000, 900, 850, 800, 750, or 700 fibers. The spinnerette may be operated at any speed suitable to produce filaments and bundles having desired size and shape.

Multiple bundles may be assembled into a CA filament yarn, such as a crimped or uncrimped tow band. As used herein, a "filament yarn" or "tow yarn" refers to a yarn formed from a plurality of continuous, untwisted individual filaments. The filament yarn may be of any suitable size and, in some embodiments, may have a total denier of at least 20,000, 25,000, 30,000, 35,000, 40,000, 45,000, 50,000, 75,000, 100,000, 150,000, 200,000, 250,000, 300,000, 350,000, 400,000, 450,000, or 500,000. Alternatively, or in addition, the total denier of the filament yarn can be no more than 5,000,000, 4,500,000, 4,000,000, 3,500,00, 3,000,000, 2,500,000, 2,000,000, 1,500,000, 1,000,000, 900,000, 800,000, 700,000, 600,00, 500,000, 400,000, 350,000, 300,000, 250,000, 200,000, 150,000, 100,000, 95,000, 90,000, 85,000, 80,000, 75,000, or 70,000.

The individual filaments, which are extruded in a generally longitudinally aligned manner and which ultimately form the filament yarn, may also be of any suitable size. For example, each filament may have a linear denier per filament (weight in grams of 9000 m fiber length) of at least 0.1, or at least 0.5, or at least 0.8, or at least 1, or at least 1.2, or at least 1.5, or at least 1.6, or at least 1.7, or at least 1.8, or at least 1.9, or at least 2.0, or at least 2.1, or at least 2.2, or at least 2.3, or at least 2.4, or at least 2.5, and/or not more or less than 3, or not more than 2.9, or not more than 2.8, or not more than 2.75, or not more than 2.6, or not more than 2.5, or not more than 2.4, or not more than 2.3, or not more than 2.2, or not more than 2.0, or not more than 1.9, measured according to ASTM D1577-01 using the FAVIMAT vibroscope procedure. Examples of ranges include 0.1 to 3.0, or 0.8 to 2.8, or 1 to 2.5, or 1 to 2.3, or 1 to 2.2, or 1 to 2.0, or 1 to 1.9, or 1.2 to 2.3, or 1.2 to 2.1, or 1.2 to 1.9, or 1.5 to 2.2, or 1.5 to less than 2.0, etc. As used herein, the term "filament" refers to an elongated, continuous single strand fiber and is distinguished from a staple fiber, which has been cut to a specified length, as described in further detail below. The staple fibers, however, will have the same dpf as the continuous filaments from which they are cut. The CA staple fibers may have a denier per filament (DPF) falling within one or more of the above minimums, maximums, or ranges (e.g., less than 3.0, 0.5 to less than 3.0, 1.0 to 2.5, or 1.5 to 2.0, etc.).

Depending on the type of application, the fiber blend may contain a blend of CA staple fibers with two or more different DPFs that are less than 3.0. For example, the fiber blend can contain a combination of CA staple fibers having a DPF from more than 2.0 to 3.0 and having a DPF of not more than 2.0. This allows one to balance the fitness for use requirements with emphasis on loft or insulation or good hand feel.

The individual filaments discharged from the spinnerette may have any cross-sectional shape. Exemplary such cross-sectional shapes include, but are not limited to, round, Y-shaped, I-shaped (dog bone), hollow, tri-lobal, multi-lobal, X-shaped, or crenulated. When a filament has a multi-lobal cross-sectional shape, it may have at least 4, 5, or 6 or more lobes. In some cases, the filaments may be symmetric along one or more, two or more, three or more, or four or more axes, and, in other embodiments, the filaments may be asymmetrical. In some cases, the CA staple fibers may be Y-shaped or tri-lobal. As used herein, the term "cross-section" or variations thereof generally refer to the transverse cross-section of the filament measured in a direction perpendicular to the direction of elongation of the filament. The cross-section of the filament may be determined and measured using Quantitative Image Analysis (QIA). Staple fibers may have a cross-sectional shape similar to the filaments from which they were formed.

The cross-sectional shape of an individual filament (or staple fiber) may be characterized according to its deviation from a round cross-sectional shape. In some cases, this deviation can be characterized by the shape factor of the filament or fiber, which is determined by the following formula: Shape Factor = Perimeter / (4π x Cross-Sectional Area)^{1/2}. In some embodiments, the shape factor of the individual CA filaments or fibers can be at least 1.0, or 1.01, 1.1, 1.15, 1.2, 1.25, 1.3, 1.35, 1.4, 1.45, 1.5, 1.55, 1.6, 1.65, 1.7, 1.75, 1.8, 1.85, 1.9, 1.95, 2, 2.25, 2.5, 2.75, 3, or 3.25 and/or not more than 5, 4.8, 4.75, 4.5, 4.25, 4, 3.75, 3.5, 3.25, 3, 2.75, 2.5, 2.25, 2, 1.75, 1.5, or 1.25. (Note: these values may also be expressed as ratios of the listed numbers to 1 - *e.g.,* 1.45:1.) The shape factor of filament or fiber having a perfectly round cross-sectional shape is 1. The shape factor can be calculated from the cross-sectional area of a filament or fiber, which can be measured using QIA.

In one embodiment or in combination with any mentioned embodiments, the CA staple fibers have a non-round shape. For example, the staple fibers can have a shape factor that is greater than 1.8, or at least 1.9, or at least 2.0, or at least 2.1, or at least 2.2. A non-round shape can enhance the insulation value of the batting as well as initial loft in applications where these features are more desirable than optimizing good hand feel. A hollow fiber can also enhance the insulation value of the batting.

Additionally, the cross-sectional shape of the CA filament or fiber may also be compared to a round cross-section according to its equivalent diameter, which is the equivalent diameter of a round filament or fiber having a cross-sectional area equal to a given filament or fiber. In some embodiments, the CA filaments or fibers can have an equivalent diameter of at least 0.0022, 0.0023, 0.0024, 0.0025, 0.0030, 0.0033, 0.0035, 0.0040, 0.0045, 0.0050, 0.0055, 0.0060, 0.0065, 0.0070, 0.0073, 0.0075, 0.0080, 0.0085, 0.0090, 0.0095, 0.0100, 0.0103, 0.0104, 0.0105, 0.0110, 0.0112, 0.0115, 0.0120, 0.0125, 0.0126, 0.013, 0.014, or 0.015 mm. Alternatively, or in addition, the CA filaments or fibers may have an equivalent diameter of not more than 0.0400, 0.0375, 0.036, 0.0359, 0.0350, 0.0033, 0.0327, 0.0325, 0.0300, 0.0275, 0.0250, 0.0232, 0.0225, 0.0200, 0.0179, 0.0175, 0.016, 0.0150, 0.0127, 0.0125, or 0.0120 mm. The equivalent diameter is calculated from the cross-section of a filament or fiber, measured using QIA.

The CA filament yarn (or tow yarn) may be passed through a crimping zone where a patterned wavelike shape is imparted to at least a portion, or substantially all, of the individual filaments.

The crimping zone includes at least one crimping device for mechanically crimping the CA tow band or yarn. An example of a mechanical crimper includes a "stuffing box" or "stuffer box" crimper that uses a plurality of rollers to generate friction, which causes the fibers to buckle and form crimps inside the box. Other types of crimpers may also be used. Examples of equipment suitable for imparting crimp to a filament yarn are described in, for example, U.S. Patent Nos. 9,179,709; 2,346,258; 3,353,239; 3,571,870; 3,813,740; 4,004,330; 4,095,318; 5,025,538; 7,152,288; and 7,585,442. In some cases, the crimping step may be performed at a rate of at least 50, 75, 100, 125, 150, 175, 200, 225, or 250 meters per minute (m/min) and/or not more than 750, 600, 550, 500, 475, 450, 425, 400, 375, 350, 325, or 300 m/min.

In some cases, low crimp, low denier per filament of CA fibers may be formed that exhibit minimal breakage and a high degree of retained tenacity. As used herein, the term "retained tenacity" refers to the ratio of the average tenacity of a crimped filament (or fiber) to the average tenacity of an identical but uncrimped filament (or fiber), expressed as a percent. For example, a crimped fiber having a tenacity of 1.3 gram-force/denier (g/denier) would have a retained tenacity of 87 percent if an identical but uncrimped fiber had a tenacity of 1.5 g/denier.

In some embodiments, crimped CA filaments may have a retained tenacity of at least 50, 55, 60, 65, 70, 75, 80, 85, 90, 95, 97, or 99 percent. Additionally, or in the alternative, the retained tenacity of the CA filaments may be no more than 99, 97, 95, 90, 92, 90, 87, 85, 82, or 80 percent, calculated as described herein. The retained tenacity may be 100 percent in some cases. Crimped filaments exhibiting a retained tenacity in these ranges is unexpected in light of the inherent weakness of most cellulose acetate filaments. In some cases, the final cellulose acetate staple fibers may exhibit similar retained tenacities as compared to identical but uncrimped staple fibers.

Crimping is performed such that the final staple fibers have a crimp frequency of at least 1, 2, 3, 4, 5, 6, 7, 8, 9, 10, 11, 12, 13, or 14 and/or not more than 30, 29, 28, 27, 26, 25, 24, 23, 22, 21, 20, 19, 18, 17, 16, 15, 14, 13, 12, 10, 9, 8, 7, or 6 crimps per inch (CPI), measured according to ASTM D3937. Examples of suitable staple fiber CPI include 1-30, 2-25, 5-25, 6-25, 6 -20, 6-18, 6-12, 8-25, 8-20, 8-18, 8-14, etc.). These values are also applicable to the filaments and yarns from which the staple fibers are cut. Measurements taken on staple fibers can be extrapolated to a CPI value based on the number of crimps present on a staple fiber and its cut length.

In one embodiment or in combination with any mentioned embodiments, the staple fibers and filaments from which they are cut are crimped. For example, the staple fibers can have a CPI shape factor that is greater than 1.8, or at least 1.9, or at least 2.0, or at least 2.1, or at least 2.2. Crimping can enhance the insulation value of the batting as well as initial loft in applications where these features are more desirable than optimizing good hand feel.

According to some embodiments, the ratio of the crimp frequency to the linear denier per filament of the individual CA filaments can be greater than 2.75:1, 2.80:1, 2.85:1, 2.90:1, 2.95:1, 3.00:1, 3.05:1, 3.10:1, 3.15:1, 3.20:1, 3.25:1, 3.30:1, 3.35:1, 3.40:1, 3.45:1, or 3.50:1. In some cases, this ratio may be even higher, such as, for example, greater than 4:1, 5:1, 6:1, 7:1, 8:1, 9:1 or even 10:1 particularly when, for example, the filaments being crimped are relatively fine.

The crimp amplitude of the CA fibers or filaments may vary and can be, for example, at least 0.85, 0.90, 0.91, 0.92, 0.93, 0.94, 0.95, 0.96, 0.97, 0.98, 0.99, 1.00, 1.01, 1.02, 1.03, 1.04, or 1.05 mm. Additionally, or in the alternative, the crimp amplitude of the fibers or filaments may be ot than 1.75, 1.70, 1.65, 1.60, 1.58, 1.55, 1.50, 1.45, 1.40, 1.37, 1.35, 1.30, 1.29, 1.28, 1.27, 1.26, 1.25, 1.24, 1.23, 1.22, 1.21, 1.20, 1.19, 1.18, 1.17, 1.16, 1.15, 1.14, 1.13, 1.12, 1.11, 1.10, 1.09, 1.08, 1.07, 1.06, 1.05, 1.04, 1.03, 1.02, 1.01, 1.00, 0.99, 0.98, 0.97, 0.96, 0.95, 0.94, 0.93, 0.92, 0.91, or 0.90 mm.

Additionally, the staple CA staple fibers or filaments from which they are cut may have a crimp ratio of at least 1:1. As used herein, "crimp ratio" refers to the ratio of the non-crimped length of the fiber or filament to the crimped length of the fiber or filament. In some embodiments, the fibers or filaments may have a crimp ratio of at least 1:1, 1.025:1, 1.05:1, 1.075:1, 1.1:1, 1.125:1, 1.15:1, 1.16:1, 1.175:1, 1.2:1, 1.225:1, 1.23:1, 1.25:1, 1.275:1, 1.3:1, 1.325:1, 1.35:1, 1.375:1, 1.39:1, 1.4:1. Additionally, or in the alternative, the CA crimped tow or staple fibers may have a crimp ratio of no more than 2.01:1, 2:1, 1.975:1, 1.95:1, 1.925:1, 1.9:1, 1.875:1, 1.85:1, 1.825:1, 1.8:1, 1.775:1, 1.75:1, 1.725:1, 1.7:1, 1.675:1, 1.65:1, 1.625:1, 1.6:1, 1.575:1, 1.55:1, 1.525:1, 1.5:1, 1.475:1, 1.45:1, 1.425:1, 1.4:1, 1.39:1, 1.375:1, or 1.35:1.

After crimping, the CA filament yarn may further be dried in a drying zone in order to reduce the moisture and/or solvent content of the filament yarn. In some cases, the drying performed in the drying zone may be sufficient to reduce the final moisture content of the filament yarn to at least 3.5, 4, 4.5, 5, 5.5, 6, 6.5, or 7 weight percent, based on the total weight of the filament yarn and/or not more than 9, 8.5, 8, 7.5, 7, or 6.5 weight percent. Any suitable type of dryer can be used in the drying zone such as, for example, a forced air oven, a drum dryer, or a heat setting channel. The dryer may be operated at any temperature and pressure conditions that provide the requisite level of drying without damaging the filament yarn. A single dryer may be used, or two or more dryers may be used in parallel or in series to achieve the desired final moisture content.

Once dried, the CA filament yarn may be baled in a baling zone, and the resulting bales may be introduced into a cutting zone, where the filament yarns may be cut into staple fibers. As used herein, the term "staple fiber" refers to a fiber cut from a filament yarn that has a discrete length, which is typically less than 150 mm. In some embodiments, the CA staple fibers may be cut to a length of at least 1, 1.5, 2, 3, 4, 5, 6, 8, 10, 12, 15, 17, 20, 22, 25, 27, 30, 32, or 35 mm. Additionally, or in the alternative, the staple fibers may have a cut length of not more than 120, 115, 110, 105, 100, 95, 90, 85, 80, 75, 70, 65, 60, 55, 51, 50, 45, 40, 35, 30, 25, 20, 10, 8, 6, 5, 4, or 3 mm. The cut length of the CA staple fibers may also fall within one or more of the above ranges (e.g., 3 to 65, 3 to 50, 6 to 55, or 10 to 51 mm). Any suitable type of cutting device may be used that is capable of cutting the filaments to a desired length without excessively damaging the fibers. Examples of cutting devices can include, but are not limited to, rotary cutters, guillotines, stretch breaking devices, reciprocating blades, and combinations thereof. Once cut, the staple fibers may be baled or otherwise bagged or packaged for subsequent transportation, storage, and/or use. The cut length of the staple fibers may be measured according to ASTM D-5103.

The CA staple fibers (or filament yarns used to form such fibers) may be at least partially coated with at least one fiber finish. As used herein, the terms "fiber finish" and "finish" refer to any suitable type of coating that, when applied to a fiber, modifies friction exerted by and on the fiber, and alters the ability of the fibers to move relative to one another and/or relative to a surface. Finishes are not the same as adhesives, bonding agents, or other similar chemical additives which, when added to fibers, prevent movement between the fibers by adhering them to one another. Finishes, when applied, continue to permit the movement of the fibers relative to one another and/or relative to other surfaces, but may modify the ease of this movement by increasing or decreasing the frictional forces. In some cases, finishes may not modify the frictional forces between fibers, but can, instead, impart one or more other desirable properties to the final coated fiber.

In some embodiments, the CA staple fibers may include at least two finishes applied to all or a portion of the staple fiber surface at one or more points during the fiber production process. In other cases, the staple fibers may only include one finish while, in other cases, the fibers may not include any finish at all. When two or more finishes are applied to the fibers, the finishes may be applied as a blend of two or more different finishes, or the finishes may be applied separately at different times during the process. For example, in some cases, the staple fibers may be at least partially coated with a spinning or spin finish applied to the filament yarn at one or more points during the process of forming the staple fibers. For example, in some embodiments, the spinning finish may be added to the fiber just after spinning. Alternatively, or in addition, the spinning finish may be added to the filament yarn just prior to the crimping step or anywhere between the spinning and crimping steps. In some cases, no spinning finish may be applied.

Any suitable method of applying the spinning finish may be used and can include, for example, spraying, wick application, dipping, or use of squeeze, lick, or kiss rollers. When used, the spinning finish may be of any suitable type and can be present on the filaments or staple fibers in an amount of at least 0.05, 0.10, 0.15, 0.20, 0.25, 0.30, 0.35, 0.40, 0.45, 0.50, 0.55, 0.60, 0.70, 0.80, 0.90, or 1 percent finish-on-yarn (FOY). Alternatively, or in addition, the spinning finish may be present in an amount of not more than 1.5, 1.4, 1.3, 1.2, 1.1, 1.0, 0.90, 0.80, 0.75, 0.70, 0.65, 0.60, or 0.50 percent finish-on-yarn (FOY) based on the total weight of the dried fiber. As used herein "FOY" or "finish on yarn" refers to the amount of finish on the staple fiber or filament, yarn less any added water. One or two or more types of spinning finishes may be used. In some cases, the spinning finish may be hydrophobic.

Additionally, or in the alternative, the CA staple fibers may include a top-coat finish added after crimping to impart certain properties or characteristics to the filaments. The top-coat finish may be added at one or more points during the formation of the staple fibers, including, for example, after the crimper, before the cutter, or after the cutter. When applied, the total amount of top-coat finish on the staple fibers or filament yarn may be at least 0.05, 0.10, 0.15, 0.20, 0.25, 0.30, or 0.35 and/or not more than 7, 6.5, 6, 5.5, 5, 4.5, 4, 3.5, 3, 2.5, 2, 1.5, 1.4, 1.3, 1.2, 1.1, 1.0, 0.90, 0.80, 0.75, 0.70, 0.65, 0.60, 0.55, 0.50, 0.45, 0.40, 0.35, 0.30, or 0.25 percent FOY, based on the total weight of the dried fiber or filament yarn. The fiber may include one or two or more types of top-coat finishes. In some embodiments, no top-coat finish may be used, while, in other embodiments, the top-coat finish may be applied even when no spinning finish is applied. In some embodiments when no spinning finish is applied, the fiber may include at least one ionic top-coat finish and may include not more than 0.05, 0.01, or 0.005% FOY, or 0% FOY of a mineral oil-based finish.

The top-coat finish may be ionic or non-ionic, and when ionic can be a cationic or an anionic finish. The finish may be in the form of a solution, an emulsion, or a dispersion. The top-coat finish may be applied to the fibers or filament yarn according to any known method, including those discussed previously with respect to the spinning finish. In some embodiments, the top-coat finish may be an aqueous emulsion and it may or may not include any type of hydrocarbon, oil including silicone oil, waxes, alcohol, glycol, or siloxanes. Examples of suitable top-coat finishes can include, but are not limited to, phosphate salts, sulfate salts, ammonium salts, and combinations thereof. Minor amounts of other components, such as surfactants, may also be present in order to enhance the stability and/or processability of the finish, and/or to make it more desirable for the intended end use of the fiber (e.g., non-irritating when the fiber will be contacted with a user's skin). Further, depending on the end use of the coated staple fibers, the finish may be compliant with various Federal and state regulations and can be, for example, non-animal, Proposition 65 compliant, and/or FDA food contact approved.

The specific type of top-coat finish applied to the CA filaments or fibers may depend, at least in part, on the final application for which the staple fibers will be used. In some embodiments, the top-coat finish may enhance the frictional forces between the fibers (or filaments) and/or with other surfaces that contact the fiber (or filaments), while, in other embodiments, the frictional forces between fibers and/or other surfaces may be reduced by the top-coat finish. Additionally, the finishes may impact the interaction of the coated fiber with water by modifying the hydrophilicity or hydrophobicity of the uncoated fiber to make it more or less hydrophilic or more or less hydrophobic. Use of a top-coat finish may or may not impart additional moisture to the fiber itself. In some embodiments, addition of the top-coat finish results in less than 1.0, 0.90, 0.80, 0.70, 0.60, 0.50, 0.40, 0.30, or 0.20% FOY moisture added to the uncoated fiber or filament.

In some cases, top-coat finishes that enhance CA fiber-to-fiber friction as compared to an identical but uncoated CA fiber may be desirable for fibers of relatively low (e.g., not more than 8 CPI) or no crimp frequency, while, in other cases, fibers having relatively higher crimp frequency (e.g., 16 CPI or higher) may benefit from top-coat finishes that either do not modify or reduce fiber-to-fiber friction as compared to an identical but uncoated fiber. In some cases, CA fibers having a crimp frequency in the range of from 8 to 16 CPI or 10 to 14 CPI may be processed with no top-coat finish. In some cases, only a top-coat finish may be applied to the fibers.

Further, in some embodiments, the top-coat (and/or spinning) finish may include other additives such as, for example, an anti-static agent. In addition, the finish may also include one or more other additives such as a wetting agent, antioxidants, biocides, anti-corrosion agents, pH control agents, emulsifiers, and combinations thereof. It is also possible that one or more additives may be added to a fiber as a coating, but without additional friction-modifying properties. For example, an antistatic agent may be applied to a fiber that does not otherwise include a top-coat finish and may be suitably formed into a nonwoven web as described herein.

When present, any suitable anti-static agent may be used. In some cases, the anti-static agent may include polar and/or hydrophilic compounds. When used, such additives may be present in any suitable amount such as, for example, at least 0.10, 0.15, 0.20, 0.25, 0.30, or 0.35 weight percent and/or not more than 3, 2.9, 2.8, 2.7, 2.6, 2.5, 2.4, 2.3, 2.2, 2.1, 2.0, 1.9, 1.8, 1.7, 1.6, 1.5, 1.4, 1.3, 1.2, 1.1, 1, 0.90, 0.80, 0.70, 0.60, or 0.50 weight percent, based on the total weight of the finish.

When the CA staple fibers are coated with an anti-static finish, the coated CA fiber may exhibit a static half-life of not more than 100, 90, 80, 75, 70, 65, 60, 55, 50, 45, 40, 35, 30, 25, 22, 20, 17, 15, 12, 10, 8, 5, 3, 2, 1.5, or 1 second, measured according to AATCC 84-2011. In some embodiments, the staple fibers may have a static half-life of not more than 30, 25, 20, 18, 15, 12, 10, or 8 minutes. In other embodiments, the static half-life of the coated fiber may be at least 30 seconds, at least 1 minute, at least 5, 8, 10, 15, 20, 30, 40, 50, 60, 75, 90, or 100 minutes and/or not more than 120, 110, 100, 90, 75, 60, 45, 40, 35, 30, 20, 15, or 12 minutes, measured according to AATCC 84-2011.

In some embodiments, this may be not more than 95, 90, 85, 80, 75, 70, 65, 60, 55, 50, 45, 40, 35, 30, 25, 20, 15, 10, or 5 percent of the static half-life of an identical but uncoated fiber. In some cases, the static half-life of the coated fiber may be at least 5, 10, 15, 20, 25, 30, 35, 40, 45, 50, 55, 60, 65, 70, 75, 80, 85, 90, or 95 percent less than the static half-life of an identical but uncoated fiber.

Alternatively, or in addition, the coated CA staple fibers may have a surface resistivity (Log R) of at least 2, 2.5, 3, 3.5, 4, 4.5, 5, 5.5, 6, 6.5, 7, 7.5, 8, 8.5, or 9 and/or not more than 11, 10.5, 10, 9.75, 9.5, 9.25, 9, 8.75, 8.5, 8.25, 8, 7.75, 7.5 measured according to AATCC TM76-2011. The surface resistivity was measured using a Monroe Electronics resistivity meter (Model No. 272A) connected to a Keithley Instruments isolation box (Model No. 6104) using an isolation cup for measuring the resistivity of the staple fibers. The surface resistivity (Log R) is calculated by multiplying the surface resistance by the ratio of the length of the area being tested to its width and expressing the result as the base 10 logarithm of the calculated value.

In some embodiments, the CA staple fibers or filament yarns may be at least partially coated with at least one spinning finish and at least one top-coat finish. The total amount of all finishes present on the staple fibers or filament yarns can be at least 0.15, 0.20, 0.25, 0.30, 0.35, 0.40, 0.45, 0.50, 0.55, 0.60, 0.65, 0.70, 0.75, 0.80, 0.85, 0.90, 0.95, 1.0, or 1.05 percent FOY and/or not more than 10, 9, 8, 7, 6, 5, 4, 3, 2, 1.5, 1.4, 1.3, 1.2, 1.1, 1.0, 0.90, 0.80, 0.75, 0.70, 0.65, 0.60, 0.55, 0.50, or 0.45 percent FOY, based on the total weight of the dried fiber. The amount of finish on the fibers as expressed by weight percent may be determined by solvent extraction according to ASTM D2257.

The coated CA staple fibers may exhibit a fiber-to-fiber (F/F) staple pad coefficient of friction (SPCOF) of at least 0.10, 0.15, 0.20, 0.25, 0.30, 0.32, 0.35, 0.40, 0.42, 0.45, 0.50, 0.55 and/or not more than 1, 0.95, 0.90, 0.85, 0.80, 0.75, 0.70, 0.65, 0.60, 0.55, 0.50, 0.45, 0.40, or 0.35, measured as described in U.S. Patent No. 5,683,811, modified as below.

A staple pad of the CA fibers whose friction is to be measured is sandwiched between a weight on top of the staple pad and a base that is underneath the staple pad and is mounted on the lower crosshead of an Instron 5966 Blue Hill machine (product of Instron Engineering Corp., Canton, Mass) with Series IX software. The staple pad is prepared by carding the staple fibers (using a roller top laboratory card) to form a batt which is cut into sections, that are 12 ins in length and 3 ins wide, with the fibers oriented in the length dimension of the batt. Enough sections are stacked up so the staple pad weighs 3 g. The metal weight on top of the staple pad is of length (L)100 mm, width (W) 45 mm, and height (H) 40 mm, and weighs 1200 gm. The surfaces of the weight and of the base that contact the staple pad are covered with 60 GC sandpaper attached with doubled sided tape, so that it is the sandpaper that contacts the surfaces of the staple pad. The staple pad is placed on the base. The weight is placed on the middle of the pad. A nylon monofil line is attached to one of the smaller vertical (W×H) faces of the weight and passed around a small pulley up to the upper crosshead of the Instron, making a 90 degree wrap angle around the pulley.

A computer interfaced to the Instron is given a signal to start the test. The lower crosshead of the Instron is moved down at a speed of 150 (+/- 30) mm/min. The staple pad, the weight and the pulley are also moved down with the base, which is mounted on the lower crosshead. Tension increases in the nylon monofil as it is stretched between the weight, which is moving down, and the upper crosshead, which remains stationary. Tension is applied to the weight in a horizontal direction, which is the direction of orientation of the fibers in the staple pad. Initially, there is little or no movement within the staple pad. The force applied to the upper crosshead of the Instron is monitored by a load cell and increases to a threshold level, when the fibers in the pad start moving past each other. Because of the Emery cloth at the interfaces with the staple pad, there is little relative motion at these interfaces; essentially any motion results from fibers within the staple pad moving past each other. The highest friction force level indicates what is required to overcome the fiber-to-fiber static friction and is recorded. The lowest friction force is the dynamic friction force. The average friction force is the average of static and dynamic friction force.

Four values are used to compute the average friction force (average load at 20-60 mm peel extension). The staple pad fiber-to-fiber coefficient of friction is determined by dividing the measured average friction force by the 1200 gm weight. The scroop value could be determined as the difference between static and dynamic friction force.

In some cases, when the CA filament yarn is coated with a spinning and/or top-coat finish, the filament yarn may exhibit a fiber-to-fiber (F/F) coefficient of friction (COF) of at least 0.01, 0.02, 0.03, 0.04, 0.05, 0.06, 0.10, 0.15, 0.20, 0.25, 0.30, 0.35, or 0.40 and/or not more than 0.55, 0.50, 0.45, 0.42, 0.40, 0.35, 0.33, 0.30, 0.25, 0.20, 0.15, 0.14, 0.13, 0.12, 0.11, 0.10, 0.09, 0.08, 0.07, or 0.06. Values for the F/F coefficient of friction (COF) of continuous filaments can be determined according to ASTM D3412 with the specified yarn parameters, a speed of 100 m/min, an input tension of 10 grams, and a single twist applied to the filament.

In one embodiment or in combination with any mentioned embodiments, CA yarns may have a F/F coefficient of friction value within one or more of the above ranges measured using a continuous tension tester electronic device (CTT-E) according to ASTM D3412 with the specified yarn parameters, a speed of 20 m/min, an input tension of 10 grams, and a single twist applied to the filament.

The fiber-to-fiber cohesion of the coated CA staple fibers may be described by the "scroop value," exhibited by the coated fiber. The scroop value, measured as the difference between static and dynamic pulling forces, of the coated fibers described herein can be less than 160 grams-force (g). In some embodiments, the coated staple fibers may exhibit a scroop value of at least 10, 15, 20, 25, 30, 35, 40, 45, 50, 55, 60, 65, 70, 75, 80, 85, 90, 95, 100, 105, 110, 115, 120, or 150 grams-force (gf) and/or not more than 275, 250, 200, 195, 190, 185, 180, 175, 170, 165, 160, 155, 150, 145, 140, 135, 130, 125, 120, 115, 110, 105, or 100 gf. Coated staple fibers with lower cohesion, as indicated by a lower scoop values, may form nonwoven materials with an overall softer feel.

The static and dynamic friction (in gram-force) and the resulting scroop value may be calculated from the staple pad friction method described in U.S. Patent Nos. 5,683,811 and 5,480,710, but using an Instron 5500 series machine, rather than an Instron 1122 machine. The fiber-to-fiber static friction is determined as described in the '710 patent as the maximum threshold pulling force at low pulling speed upon reaching equilibrium pulling behavior, and the fiber-to-fiber dynamic friction is similarly calculated, but is the minimum threshold level of force as the staple pad traverses a slip-stick behavior. The scroop is calculated as the difference between static and dynamic friction pulling forces with units of gram-force.

The coated CA staple fibers may also exhibit high strength. For example, in some embodiments, the coated staple fibers may be formed from filaments that exhibit a tenacity of at least 0.5, 0.55, 0.60, 0.65, 0.70, 0.75, 0.80, 0.85, 0.90, 0.95, 1.0, 1.05, 1.1, 1.15, 1.20, 1.25, 1.30, or 1.35 grams-force/denier (g/denier) and/or not more than 2.50, 2.45, 2.40, 2.35, 2.30, 2.25, 2.20, 2.15, 2.10, 2.05, 2.00, 1.95, 1.90, 1.85, 1.80, 1.75, 1.70, 1.65, 1.60, 1.55, 1.50, 1.47, 1.45, or 1.40 g/denier, measured according to ASTM D3822. Additionally, in some embodiments, the elongation at break of the coated staple fibers (or filaments from which the staple fibers are formed) can be at least 5, 6, 10, 15, 20, or 25 percent and/or not more than 50, 45, 40, 35, or 30 percent, measured according to ASTM D3822.

Traditionally, CA fibers and filaments are coated with a plasticizer in order to facilitate formation and ultimate biodegradability of the final fibrous article. However, the fibers and filament yarns can include little or no plasticizer and can unexpectedly exhibit enhanced biodegradability under industrial, home, and soil conditions, even as compared to cellulose acetate fibers with higher levels of plasticizer.

In some embodiments, the CA fibers can include not more than 30, 27, 25, 22, 20, 17, 15, 12, 10, 9.5, 9, 8.5, 8, 7.5, 7, 6.5, 6, 5.5, 5, 4.5, 4, 3.5, 3, 2.5, 2, 1.5, 1, 0.5, 0.25, or 0.10 percent of plasticizers, based on the total weight of the fiber, or the fibers may include no plasticizer. When present, the plasticizer may be incorporated into the fiber itself by being blended with the solvent dope or cellulose acetate flake, or the plasticizer may be applied to the surface of the fiber or filament by spraying, by centrifugal force from a rotating drum apparatus, or by an immersion bath.

Examples of plasticizers that may or may not be present in or on the fibers can include, but are not limited to, aromatic polycarboxylic acid esters, aliphatic polycarboxylic acid esters, lower fatty acid esters of polyhydric alcohols, and phosphoric acid esters. Further examples can include, but are not limited to, dimethyl phthalate, diethyl phthalate, dibutyl phthalate, dihexyl phthalate, dioctyl phthalate, dimethoxyethyl phthalate, ethyl phthalylethyl glycolate, butyl phthalylbutyl glycolate, tetraoctyl pyromellitate, trioctyl trimellitate, dibutyl adipate, dioctyl adipate, dibutyl sebacate, dioctyl sebacate, diethyl azelate, dibutyl azelate, dioctyl azelate, glycerol, trimethylolpropane, pentaerythritol, sorbitol, glycerin triacetate (triacetin), diglycerin tetracetate, triethyl phosphate, tributyl phosphate, tributoxyethyl phosphate, triphenyl phosphate, and tricresyl phosphate, and combinations thereof. In some embodiments, the CA fibers may not include any type of plasticizer or other additive, and can consist essentially of, or consist of, CA and not more than 1 percent FOY of a spinning finish.

Additionally, the CA fibers may not have undergone additional treatment steps designed to enhance the biodegradability of the fibers. For example, the fibers may not have been hydroylzed or treated with enyzmes or microorganisms. The fibers may include not more than 1, 0.75, 0.5, 0.25, 0.1, 0.05, or 0.01 weight percent of an adhesive or bonding agent and may include less than 1, 0.75, 0.5, 0.25, 0.1, 0.05, or 0.01 weigh percent of modified or substituted cellulose acetate. In some embodiments, the fibers may not include any adhesive or bonding agent and may not be formed from any substituted or modified CE. Substituted or modified CA may include CA that has been modified with a polar substituent, such as a substituent selected from the group consisting of sulfates, phosphates, borates, carbonates, and combinations thereof.

In one embodiment or in combination with any mentioned embodiments, there is provided a blend of at least two different CA staple fibers, each having a DPF of not more than 3.0, where the difference between the at least two different CA fibers is one or more of:
a. DPF,
b. CPI, or
c. Shape.

The at least two different CA staple fibers can have two or more of the above mentioned differences. In one embodiment or in combination with any mentioned embodiments, all the CA staple fibers are non-round, and there is provided a blend of at least two different CA staple fibers, each having a different DPF.

The fiber blend also includes a structural staple fiber having a DPF of more than 6.0. The structural staple fibers can be a CA fiber, synthetic fiber, such as polyester, polyamide, Lyocell, acrylics having at least 35 wt.% acrylonitrile repeating units, or polyolefin fibers, or blends thereof, other than CA fibers or other fibers derived from a cellulose backbone such as regenerated cellulose fibers other than Lyocell. The structural staple fiber can also be glass fibers for structural insulation. The structural aspect of the fiber is primarily driven by its high DPF of at least 6.0. The high DPF structural staple fibers of CA fibers, polyolefins, acrylics, polyesters, Lyocell, and polyamides all provide good resilience to deformation or compressive forces and to washing cycles. In one embodiment or in combination with any mentioned embodiments, the fiber blend, the non-woven batting, or the fiber fill in the article, contains not more than 25 wt.%, or not more than 20 wt.%, or not more than 15 wt.%, or not more than 13 wt.%, or not more than 10 wt.%, or not more than 8 wt.%, or not more than 5 wt.%, or not more than 3 wt.%, or no added amount of silk, cotton, flax, or rayon as these fibers do not have the performance of synthetic fibers in terms of resilience, loft, and feel. For human contact applications (direct or indirect) such as apparel, the same quantity values apply to glass fibers. Among the synthetic fibers used as structural staple fibers, cellulose acetate, polyester and acrylic are desirable, and cellulose acetate and polyester are the most desirable.

In one embodiment or in combination with any mentioned embodiments, the structural staple fibers are mono-component fibers. The structural staple fibers can have any of the shapes mentioned with respect to CA fibers, and also can include hollow structural staple fibers.

Natural fibers can also be a structural staple fiber, although compared to synthetic fibers, they lag behind the dual soft feel and resilience of synthetic fibers. Among the natural fibers, cotton is the most desirable structural staple fiber as it, more than other natural fibers, approaches the feel and resilience of the synthetic fibers. In one embodiment or in combination with any mentioned embodiments, however, the fiber blend, the batting, and the non-woven articles contain not more than 25 wt.%, or not more than 15 wt.%, or not more than 10 wt.%, or not more than 5 wt.%, or not more than 2 wt.%, or no cotton, or natural fibers, based on the weight of the fiber blend, batting or non-woven article.

In one embodiment or in combination with any mentioned embodiments, the structural staple fibers (those having a dpf of 6.0 or more) include CA fibers. The structural staple fiber can include a CA fiber, or at least 25 wt.%, or at least 50 wt.%, or at least 75 wt.%, or all of the fibers having a DPF of 6.0 or more, other than binder fibers, can be CA fibers. This embodiment has the advantage in that the majority, if not all, of the fibers in the fiber fill or non-woven batting or article can be sustainably derived and biodegradable.

In one embodiment or in combination with any mentioned embodiments, the structural staple fiber does not include a CA fiber. In one embodiment or in combination with any mentioned embodiments, at least a portion, or at least 25 wt.%, or at least 50 wt.%, or at least 75 wt.%, or at least 100 wt.% of the structural staple fibers having a dpf of 6.0 or more, and other than the binder fibers, are fibers other than CA fibers, or are synthetic fibers, or are polyester or acrylic fibers.

The fiber fill can optionally include a binder fiber. A binder fiber is included when the Tg of all fibers among the CA fibers and the structural staple fibers is above 192°C. The binder fiber can be the same fiber as the structural staple fibers if the structural staple fibers have the desired Tg. Much of the thermal bonding equipment operate at lower temperatures, typically around 150 to 170°C. In most cases, the structural staple fibers will have a Tg suitable for thermally bonding with conventional equipment, in which case there is no need for an additional binding fiber since the structural staple fiber serves both purposes. If a binder fiber is added because the fiber blend selected does not include a fiber with a Tg below 192°C or a Tg at or below the temperature used in thermal bonding equipment, and in the event that one also desires to solely thermally bond the non-woven web rather than resin bind the web, a binder fiber can be added.

Any type of binder fiber can be used in the fiber blend, provided that the binder fiber (or at least a portion of it) has a Tg at or lower than the operating capabilities of the thermal bonding equipment employed using the particular blend, or lower than the glass transition temperature than that of unplasticized CA fiber, or a lower Tg than 192°C, optionally a Tg that is lower than 190°C, or lower than 185°C, or lower than 180°C, or lower than 170°C, or not more than 165°C, or not more than 160°C. Of course, if the thermal bonding equipment can operate at temperatures exceeding 192°C and the fiber blend is not damaged at those higher temperatures, there is no need for a binder fibers. The use of a binder fiber allows one to thermally bond the non-woven web without the need to use resins. During heat-setting, the binder fiber melts and bonds to the CA staple fibers at the cross-over points so that the bonded batting retains the desired configuration and density. The binder is used to give the heat-bonded batting stability and recoverable stretch. The binder fiber can be processed on conventional textile machinery, e.g. a card, and be distributed throughout the blend. It is desirable, therefore, that the DPF of the binder fiber be compatible with the denier of the CA staple fibers so that it can be distributed throughout the blend by conventional textile processing. The DPF of the binder fiber desirably is either not more than 3.0 or at least 6.0, or not more than 25%, or not more than 20%, or not more than 15%, or not more than 10% different than the CA fiber DPF or the structural staple fiber DPF. Ideally, it could be preferable to use a binder fiber of substantially the same denier as that of the CA staple fiber, but a satisfactory result can be obtained by using binder fiber having a higher or a low denier.

If a CA fiber is used as a binder fiber as either the low DPF or structural staple fiber component, it desirably has a Tg lower than its native Tg, or within any of the above stated Tg values. This can be accomplished by adding a plasticizer to the CA fiber to depress it Tg value to a value within the stated Tg ranges. The type and amount can be the amounts expressed above related to the use of plasticizers, and in addition, water can be employed in a hydroentangling process that can also plasticize the CA fibers.

Generally, binder fibers other than the structural staple fibers are not needed because the structural staple fibers can also serve as binder fibers. Typical binder fibers are made of polyesters, such as polyethylene terephthalate (PET); copolymers thereof; polyolefins, such as polypropylene and polyethylene; and mixtures thereof. In some cases, the binder fibers may be single-component fibers, while, in other cases, the fibers could be multicomponent fibers. When the binder fibers are bicomponent or multicomponent fibers, they may have any suitable cross-section, including, for example, in a side-by-side cross-section, a core-and-sheath cross-section, an islands-in-the-sea cross-section, a tipped cross-section, or a segmented pie cross-section. In some cases, the binder fiber can be a bicomponent fiber comprising a polyester (e.g., PET) and a copolyester (e.g., PETG). In some cases, the binder fiber can be a bicomponent fiber comprising a polyester (e.g., PET) and a polyolefin (e.g., PE or PP). And in some cases, the binder fiber can be a bicomponent fiber comprising a first polyolefin (e.g., PE) and a second polyolefin (e.g., PP). Specific examples of binder fibers are described in U.S. Patent Nos. 4,068,036; 4,129,675; and 4,304,817.

The binder fiber can have a cut length within any of the ranges expressed above with respect to the CA and structural staple fibers.

The amount of CA fibers having a DPF of 3.0 or less, structural staple fibers having a DPF of 6.0 or more, and optional binder fibers if used:
A. 45-60 wt.% of CA fibers having a DPF of 3.0 or less; and
B. 20-35 wt.% wt.% of a structural staple fiber having a DPF of 6.0 or more, optionally a polyester fiber, CA fiber, acrylic fiber, or a combinations thereof; and
C. optional binder fibers in an amount of 0 to 30 wt%, or 10 to 25 wt.%, of the blend,
in each case based on the weight of the fiber blend or non-woven web.

The fiber blend may be prepared by conventional blending techniques. The fiber blend may then undergo a web forming step and a web bonding step to form a thermally-bonded, nonwoven web. The web forming step may be performed under dry conditions, and the web bonding step may be carried out thermally. The web forming step may include one or more dry-laid processes. Dry-laid processes include air-laying and carding processes.

In an air-laid process, the fibers are entrained in streams of air, which are directed to a conveyor, onto which the fibers are deposited to form a web. In a carding process, fibers placed on a conveyor, or card, and are passed through a pair of rollers (or other movable surfaces) having a set of metal teeth or other gripping surfaces. As the surfaces move relative to one another, the fibers are mechanically separated and aligned to form a web.

In the event that the fiber fill contains two or more types of cellulose acetate fibers, either by the DS, their DPF, cut length, CPI, shape, or other morphological characteristic, one may simply produce bales of each of the fiber types and blend them together by withdrawing each from the bale prior to carding. Alternatively, one may set up a spinning machine with multiple different spinnerets so that multiple different filaments with different DPF's and/or cross-sections are spun, bundled, and combined within a single tow band on a continuous basis to produce mixed filament types that are then cut into staple fibers and baled to obtain bales each having a mix of different types of CA fibers (by type can be any of the differences noted above). Using this approach one may sell a pre-mixed bale of fibers that included all of the necessary fiber types that an insulation manufacturer would need to produce a batting. Rather than blending multiple different staple fiber bales together prior to carding, the manufacturer could use the pre-mixed bales to generate the battings.

In some cases, the CA staple fibers are lapped horizontally relative to the web's thickness. In other cases, after the dry-laying process, the web may be passed to a vertical lapping machine to impose a plurality of vertical parallel pleats on the web, relative to the web's thickness, which are then compressed to form a pleated web. The pleated web may be joined face-to-face with a second adhesive web to create a laminated composite web. Examples of vertical lapping machines are described in U.S. Patent Nos. 5,995,174; 7,591,049; and 9,783,915.

Once the web is formed, the web may be transported to a web bonding zone where it is heated to form a bonded web. Examples of thermal bonding methods include, but are not limited to, calendaring, ultrasonic bonding, and through-air oven bonding. Particular suitable combinations of web formation and bonding steps include, but are not limited to, formation by carding and thermal bonding or air-laying and thermal bonding.

The process for forming a nonwoven web with CA fibers as described herein may be performed on a lab-, pilot-, and/or commercial scale. It has been discovered that use of the CA fibers described herein may provide processing advantages that permit formation of nonwoven webs on a larger, commercial scale. For example, in some embodiments, the web forming step may be carried out at a rate of at least 50, 75, 100, 125, 150, 175, 200, 225, 250, 275, 300, 325, 350, 375, 400, 425, 450, 475, or 500 meters per minute (m/min). Additionally, or in the alternative, the web forming step may be performed at a rate of not more than 600, 575, 550, 525, 500, 475, 450, 425, 400, 375, 350, 325, or 300 m/min.

In some embodiments, the nonwoven web can have a thickness of at least 0.25, 0.30, 0.35, 0.40, 0.45, 0.50, 0.55, 0.60, 0.65, 0.70, 0.75, 0.80, 0.85, 0.90, or 0.95 mm and/or not more than 2.75, 2.5, 2.25, 2.0, 1.9, 1.8, 1.7, 1.6, 1.5, 1.4, 1.3, 1.2, 1.1, 1.05, 0.95, 0.90, 0.85, 0.80, 0.75, 0.70, 0.65, 0.60, 0.55, or 0.50 mm. In some cases, the thickness of the nonwoven web can be at least 20, 30, 40, 50, 60, 70, 80, 90, 100, 125, 150, 175, or 200 mm and/or not more than 400, 375, 350, 325, 300, 275, 250, 225, 200, 175, 150, 125, 100, 90, 80, 70, 60, 50, 40, 30, or 20 mm. Thickness can be measured according to NWSP 120.1.R0 (15).

The nonwoven web may have a basis weight of at least 15, 20, 25, 30, 35, 40, 45, 50, 51, 52, 53, 54, 55, 56, 57, 58, 59, 60, 61, or 62 grams per square meter (gsm) and/or not more than 80, 75, 74, 73, 72, 71, 70, 69, 68, 67, 66, 65, 64, 63, or 62 gsm. In some cases, the nonwoven webs can have a basis weight of at least 50, 75, 100, 125, 150, 175, 200, 225, 250, 275, 300, 325, 350, 375, 400, 425, 450, 475, 500, 525, 550, 575, 600, 700, 800, 900, or 1000 gsm. Alternatively, or in addition, the nonwoven web may have a basis weight of not more than 8000, 7500, 7000, 6500, 6000, 5500, 5000, 4500, 4000, 3500, 3000, 2500, 2000, 1500, 1000, 500, 400, 300, 200, or 150 gsm. Basis weight can be measured according to NWSP 130.1.R0 (15).

According to some embodiments, the nonwoven web can exhibit one or more of the following characteristics: (i) a wet tensile strength in the machine direction (MD) in the range of 10 to 2000 Nm²/kg, normalized for the basis weight of the nonwoven; (ii) a wet tensile strength in the cross direction (CD) in the range of 10 to 1000 Nm²/kg, normalized for the basis weight of the nonwoven; (iii) a dry tensile strength in the machine direction (MD) in the range of 10 to 2000 Nm²/kg, normalized for the basis weight of the nonwoven; (iv) a dry tensile strength in the cross direction (CD) in the range of 10 to 1000 Nm²/kg, normalized for the basis weight of the nonwoven; an absorbency in the range of 5 to 20 grams of water per grams of fiber (g/g); and (vi) a real softness in the range of from 2.5 to 6 dB. In some cases, the nonwoven may exhibit at least two, at least three, at least four, at least five, or all of characteristics (i) through (vi) listed above.

The nonwoven web can have a dry tensile strength in the machine direction of at least 0.5, 1, 2, 5, 10, 12, 15, 20, 25, 30, 35, 40, 45, 50, 55, or 60 N/in and/or not more than 250, 245, 240, 235, 230, 225, 220, 215, 210, 205, 200, 195, 190, 185, 180, 175, 170, 165, 160, 155, 150, 145, 140, 135, 130, 125, 120, 115, 110, 100, 95, 90, 85, 90, 75, 60, 5, 50, 45, 40, 35, 30, or 25 N/in, measured according to the procedure described in NWSP 110.4 Option A with a 1-inch test strip. All tensile strength measurements are performed on a 1-inch strip of sample, unless otherwise stated.

Additionally, or in the alternative, the nonwoven web may have a dry tensile strength in the cross direction of at least 0.5, 1, 3, 4, 5, 10, 15, 20, 25, 30, 35, 40, or 45 N/in and/or not more than 225, 200, 190, 180, 175, 170, 160, 150, 140, 130, 125, 120, 110, 100, 90, 80, 75, 70, 60, 50, 45, 40, 35, 30, 25, 20, 15, 12, 10, 8, or 5 N/in, measured according to NWSP 110.4 Option A.

In some embodiments, the ratio of dry tensile strength in the machine direction to dry tensile strength in the cross direction (dry MD:CD) can be no more than 10:1, 9.5:1, 9:1, 8.5:1, 8:1, 7.5:1, 7:1, 6.5:1, 6:1, 5.5:1, 5:1, 4.5:1, 4:1, 3.5:1, 3:1, 2.5:1, 2:1, 1.5:1, 1.25:1, or 1.1:1. In some cases, the ratio of dry MD:CD can be at least 1.01:1, 1.05:1, 1.10:1, 1.15:1, 1.20:1, 1.25:1, 1.30:1, 1.35:1, 1.4:1, 1.45:1, 1.5:1, 1.55:1, 1.6:1, 1.65:1, 1.7:1, 1.75:1, 1.8:1, or 1.85:1.

The nonwoven web may have a wet tensile strength in the machine direction of at least 0.5, 1, 1.5, 5, 10, 15, 20, 25, 30, 35, 40, 45, or 50 N and/or not more than 250, 240, 230, 220, 210, 200, 190, 180, 170, 160, 150, 145, 140, 135, 130, 125, 120, 115, 110, 105, 100, 95, 90, 85, 80, 75, 70, 65, 60, 50, 40, 35, 30, 25, or 20 N/in, measured according to NWSP 110.4 Option A.

Additionally, the nonwoven web can have a wet tensile strength in the cross-direction of at least 0.5, 1, 1.5, 2, 3, 4, 5, 8, 10, 12, 15, 18, or 20 N/in and/or not more than 120, 115, 110, 105, 100, 95, 90, 85, 80, 75, 70, 65, 60, 55, 50, 45, 40, 35, 30, 28, 25, 20, 15, 12, or 10 N/in, measured according to NWSP 110.4 Option A.

In some embodiments, the ratio of wet tensile strength in the machine direction to wet tensile strength in the cross direction (wet MD:CD) can be no more than 10:1, 9.5:1, 9:1, 8.5:1, 8:1, 7.5:1, 7:1, 6.5:1, 6:1, 5.5:1, 5:1, 4.5:1, 4:1, 3.5:1, 3:1, 2.5:1, 2:1, 1.5:1, 1.25:1, or 1.1:1. In some cases, the ratio of wet MD:CD can be at least 1.01:1, 1.05:1, 1.10:1, 1.15:1, 1.20:1, 1.25:1, 1.30:1, 1.35:1, 1.4:1, 1.45:1, 1.5:1, 1.55:1, 1.6:1, 1.65:1, 1.7:1, 1.75:1, 1.8:1, or 1.85:1.

The tensile strength of the nonwoven web may be normalized according to the basis weight, thickness, and/or bulk density of the web. In some cases, the nonwoven web may have a wet tensile strength in the machine direction, normalized for the basis weight of the nonwoven, of at least 10, 20, 40, 60, 80, 100, 200, 300, 400, 500, 600, 700, 800, or 900 Nm²/kg and/or not more than 2000, 1900, 1800, 1700, 1600, 1500, 1400, 1300, 1200, 1100, 1000, 900, 800, 700, 600, 500, or 400 Nm²/kg, measured according to NWSP 110.4 Option A. Additionally, the nonwoven web may have a wet tensile strength in the cross-direction, normalized for the basis weight of the nonwoven, of at least 10, 20, 40, 60, 80, 100, 200, 240, or 250 Nm²/kg and/or not more than 1000, 900, 800, 700, 600, 560, 500, 400, or 300 Nm²/kg, measured according to NWSP 110.4 Option A.

The dry tensile strength in the machine direction, normalized according to basis weight of the nonwoven, may be at least 10, 25, 50, 100, 200, 300, 400, 500, 600, 700, 800, 900, or 1000 Nm²/kg and/or not more than 5000, 4500, 4000, 3500, 3400, 3000, 2500, 2000, 1500, 1000, 750, or 500 Nm²/kg, while the dry tensile strength in the cross direction normalized for basis weight can be at least 10, 25, 50, 80, 100, 200, 250, or 300 Nm²/kg and/or not more than 4000, 3500, 3000, 2500, 2000, 1500, 1200, 1000, 900, or 500 Nm²/kg, measured according to NWSP 100.4 Option A.

The nonwoven web may have a wet tensile strength in the machine direction, normalized for the thickness of the nonwoven, of at least 2000, 3000, 4000, 5000, 6000, 7000, 8000, 9000, 10,000, 15,000, 20,000, 25,000, 30,000, 35,000, 40,000, or 45,000 N/m and/or not more than 150,000, 145,000, 140,000, 135,000, 130,000, 125,000, 120,000, 117,000, 115,000, 110,000, 100,000, 80,000, 60,000, 40,000, or 20,000 N/m, measured according to NWSP 110.4 Option A. Additionally, the nonwoven web may have a wet tensile strength in the cross-direction, normalized for the thickness of the nonwoven, of at least 2000, 3000, 4000, 5000, 6000, 7000, 8000, 9000, 10,000, 12,000, 15,000, or 20,000 N/m and/or not more than 100,000, 95,000, 90,000, 85,000, 83,000, 80,000, 75,000, 70,000, 65,000, 60,000, 55,000, 50,000, 47,000, 45,000, or 40,000 N/m, measured according to NWSP 110.4 Option A.

The dry tensile strength in the machine direction, normalized according to the thickness of the nonwoven, may be at least 1000, 2000, 3000, 4000, 5000, 6000, 7000, 8000, 9000, 10,000, 12,000, 15,000, 20,000, 25,000, 30,000, 35,000, 40,000, 45,000, or 50,000 N/m and/or not more than 450,000, 417,000, 400,000, 350,000, 300,000, 283,000, 250,000, or 200,000 N/m, while the dry tensile strength in the cross direction normalized for thickness can be at least 3000, 4000, 5000, 6000, 7000, 8000, 9000, 10,000, 11,000, 12,000, 13,000, 14,000, or 15,000 N/m and/or not more than 400,000, 350,000, 300,000, 250,000, 200,000, 150,000, 100,000, 75,000, or 50,000 N/m, measured according to NWSP 100.4 Option A.

When normalized for the bulk density, the nonwoven web may have a wet tensile strength in the machine direction of at least 0.01, 0.05, 0.07, 0.10, 0.12, 0.15, 0.20, 0.25, 0.30, 0.35, 0.40, 0.45, 0.50, 0.54, or 0.55 Nm³/kg and/or not more than 2.0, 1.9, 1.8, 1.7, 1.6, 1.5, 1.4, 1.3, 1.2, 1.1, 1.0, 0.9, 0.8, 0.7, 0.6, 0.5, 0.4, or 0.3 Nm³/kg, measured according to NWSP 110.4 Option A. Additionally, the nonwoven web may have a wet tensile strength in the cross-direction, normalized for the bulk density of the nonwoven, of at least 0.01, 0.02, 0.05, 0.07, 0.10, 0.12, 0.15, 0.20, 0.25, 0.30, 0.35, 0.40, 0.45, 0.50, 0.54, or 0.55 Nm³/kg and/or not more than 2.0, 1.9, 1.8, 1.7, 1.6, 1.5, 1.4, 1.3, 1.2, 1.1, 1.0, 0.90, 0.80, 0.70, 0.60, 0.56, 0.50, 0.40, or 0.3 Nm³/kg, measured according to NWSP 110.4 Option A.

The dry tensile strength in the machine direction, normalized according to bulk density of the nonwoven, may be at least 0.01, 0.02, 0.05, 0.07, 0.10, 0.12, 0.15, 0.20, 0.25, 0.30, 0.35, 0.40, 0.45, 0.50, 0.55, or 0.60 Nm³/kg and/or not more than 5, 4.5, 4, 3.5, 3.4, 3, 2.5, 2, 1.5, 1, 0.5, or 0.3 Nm³/kg, while the dry tensile strength in the cross direction normalized for basis weight can be at least 0.01, 0.02, 0.05, 0.07, 0.10, 0.12, 0.15, 0.18, 0.20, 0.25, 0.30, 0.35, 0.40, 0.45, 0.50, 0.55, or 0.60 Nm³/kg and/or not more than 2.0, 1.9, 1.8, 1.7, 1.6, 1.5, 1.4, 1.3, 1.2, 1.1, 1.0, 0.90, 0.80, 0.70, 0.60, 0.56, 0.50, 0.40, or 0.3 Nm³/kg, measured according to NWSP 100.4 Option A.

In some cases, the wet bondability index (BI₂₀) of the nonwoven web can be at least 0.1, 0.2, 0.5, 1, 2, 2.5, 5, 6, 7, 8, 9, 10, 11, 12, or 13 and/or not more than 30, 29, 28, 27, 26, 25, 24, 23, 22, 21, 20, 19, 18, 17, 16, 15, 14, 13, 12, 11, 10, 9, 8, 7, 6, 5, or 4. The dry bondability index of the nonwoven can be at least 0.1, 0.5, 1, 2, 2.5, 3, 4, 5, 6, 7, 8, 9, 10, 12, 15, 17, or 20. Alternatively, or in addition, the dry bondability of the nonwoven can be no more than 50, 45, 40, 35, 30, 25, 20, 15, or 10. The bondability index of the nonwoven is defined as the square root of the product of the tensile strength in the machine direction and the tensile strength in the cross direction. The calculated bondability index is multiplied by 20 and divided by the actual base weight in g/m² to report bondability index in standard nonwovens base weight of 20g/m² (BI₂₀). The wet and dry tensile strengths are measured as described herein.

Additionally, or in the alternative, the nonwoven web may have an absorbency of at least 300 percent (3 grams of water per gram of fiber). In other embodiments, the nonwoven web may have an absorbency of at least 400, 450, 500, 550, 600, 650, 700, 750, 800, 850, 900, 950, 1000, 1050, 1100, or 1150 percent, or at least 4, 4.5, 5, 5.5, 6, 6.5, 7, 7.5, 8, 8.5, 9, 9.5, 10, 10.5, 11, or 11.5 grams of water per gram of fiber. In some embodiments, the nonwoven web may have an absorbency of not more than 2500, 2400, 2300, 2200, 2100, 2000, 1950, 1900, 1850, 1800, 1750, 1700, 1650, 1600, 1550, 1500, 1450, 1400, 1350, 1300, 1250, 1200, or 1150 percent, or not more than 25, 24, 23, 22, 21, 20, 19.5, 19, 18.5, 18, 17.5, 17, 16.5, 16, 15.5, 15, 14.5, 14, 13.5, 13, 12.5, 12, or 11.5 grams of water per gram of fiber. Absorbency values provided herein are measured as described in NWSP 010.1-7.2.

The nonwoven web may also exhibit desirable wicking properties. For example, in some embodiments, the nonwoven web may have a wicking height, measured in the cross or machine direction, at 5 minutes of not more than 200 mm. In some case, the wicking height of the nonwoven web can be no more than 200, 175, 150, 125, 100, 95, 90, 85, 80, 75, 70, 65, 60, 55, 50, 45, 40, 35, 30, 25, 20, 15, 10, or 5 mm, measured as described in NWSP 010.1-7.3. Additionally, or in the alternative, the wicking height can be at least 1, 5, 10, or 20 mm, measured as described in NWSP 010.1-7.3.

In some embodiments, the nonwoven web may have a wicking height, measured in the machine or cross direction, of at least 1, at least 2, at least 3, at least 5, at least 10, at least 12, at least 15, at least 20, at least 25, at least 30, at least 35, at least 40, at least 45, at least 50, or at least 55 mm, measured as described in NWSP 010.1-7.3. Alternatively, or in addition, the nonwoven web may have a wicking height, measured in the machine or cross direction, of not more than 70, not more than 65, not more than 60, not more than 55, not more than 50, not more than 45, not more than 40, not more than 35, not more than 30, not more than 25, not more than 20, not more than 15, not more than 12, not more than 10, not more than 8, not more than 5, not more than 3, or not more than 2 mm, measured as described in NWSP 010.1-7.3.

The fiber blend, or the nonwoven web, can exhibit superior initial thermal insulation per equivalent unit loft. In one embodiment or in combination with any mentioned embodiments, the nonwoven web can have an initial clo value per millimeter of loft of at least 0.180, or at least 0.185, or at least 0.190, or at least 0.195, or at least 0.2, or at least 0.205, or at least 0.21, or at least 0.215, or at least 0.22, or at least 0.225, or at least 0.23, or at least 0.235, or at least 0.24, or at least 0.245, or at least 0.250, and/or up to 3.0, or up to 2.9, or up to 2.85, or up to 2.8, or up to 2.75, or up to 2.7, in each case as clo/mm. The fiber blend, or the nonwoven web, can exhibit a higher initial thermal insulation per equivalent unit loft than the same fiber blend made without CA fibers having a DPF of 3.0 or less and replacing that quantity with the structural staple fiber used in the blend or web at the structural staple fiber dpf ("Comparative Blend"). In one embodiment or in combination with any mentioned embodiments, the nonwoven web can have an initial clo value per millimeter of loft that is 10% higher, or 15% higher, or 20% higher, or 30 higher, or 40% higher, or 50% higher, or 60% higher, or 70% higher, or 80% higher, than the Comparative Blend.

The "initial" value of a fiber blend or non-woven web is the measured value before the fiber fill or non-woven web is laundered or wetted.

The fiber blend, or the nonwoven web, can exhibit superior initial loft per mm. In one embodiment or in combination with any mentioned embodiments, the nonwoven web can have an initial loft/mm of at least 13 mm, or at least 13.5 mm, or at least 14 mm, or at least 14.5 mm, or at least 15 mm, or at least 15.5 mm, or at least 16 mm, or at least 16.5 mm, or at least 17 mm, or at least 17.5 mm, or at least 18 mm, or at least 18.5 mm, or at least 19 mm, and/or up to 21 mm, or up to 20 mm. The fiber blend, or the nonwoven web, can exhibit a higher initial loft per mm than a Comparative Blend. In one embodiment or in combination with any mentioned embodiments, the nonwoven web can have an initial loft per millimeter that is 10% higher, or 15% higher, or 20% higher, or 30 higher, or 40% higher, or 50% higher, or 60% higher, or 70% higher, or 80% higher, than the Comparative Blend.

The fiber blend, or the nonwoven web, can exhibit good thermal insulation per equivalent unit loft at 5 wash cycles or more. In one embodiment or in combination with any mentioned embodiments, the nonwoven web can have a clo value per millimiter of loft at 5 wash cycles of at least 0.130, or at least 0.135, or at least 0.140, or at least 0.145, or at least 0.15 or at least 0.155, or at least 0.16, or at least 0.165, or at least 0.17, or at least 0.175, or at least 0.18 and/or up to 0.20, or up to 0.195, or up to 0.19, or up to 0.185, or up to 0.18, or up to 0.175, in each case as clo/mm. These clo values, after 5 wash cycles, are comparable or better than the clo values of a Comparative Blend. In one embodiment or in combination with any mentioned embodiments, the nonwoven web can have the above stated minimum clo values per millimiter of loft even at 10 wash cycles. In one embodiment or in combination with any mentioned embodiments, the nonwoven web can have the clo values per millimiter of loft at 20 wash cycles of at least 0.120, or at least 0.125, or at least 0.130, or at least 0.135, or at least 0.140, or at least 0.145, and/or up to 0.17, or up to 0.165, or up to 0.16, or up to 0.155, in each case as clo/mm.

The fiber blend, or the nonwoven web, can exhibit good loft per mm at 5 wash cycles. In one embodiment or in combination with any mentioned embodiments, the nonwoven web can have a loft in mm at 5 wash cycles of at least 7 mm, or at least 7.5 mm, or at least 8 mm, or at least 8.5 mm, and/or up to 13 mm, or up to 12.5 mm, or up to 12 mm. The fiber blend, or the nonwoven web, can exhibit a higher initial loft per mm than a Comparative Blend. In one embodiment or in combination with any mentioned embodiments, the nonwoven web can have an initial loft per millimeter that is 10% higher, or 15% higher, or 20% higher, or 30 higher, or 40% higher, or 50% higher, or 60% higher, or 70% higher, or 80% higher, than the Comparative Blend. In one embodiment or in combination with any mentioned embodiments, the nonwoven web can have the above stated minimum loft values even at 10 wash cycles. In one embodiment or in combination with any mentioned embodiments, the nonwoven web can have the loft values at 20 wash cycles of at least 6 mm, or at least 6.5 mm, or at least 7 mm, or at least 7.5 mm, or at least 8 mm, or at least 8.5 mm, and/or up to 10 mm, or up to 9.5 mm.

In one embodiment or in combination with any mentioned embodiments, the fiber blend, or the nonwoven web, can exhibit a combination of both good loft per mm and good clo per mm. The combination can be the combination of any of the values indicated above at each of their respective initial, 5, 10 and 20 wash cycles. Thus, there is provided a fiber fill, non-woven web, batting, interliner, or any other articles mentioned that has both good loft and thermal insulation after multiple wash cycles and contains sustainable and optionally biodegradable fibers.

In one embodiment or in combination with any mentioned embodiments, the fiber blend, or the nonwoven web, can exhibit a good clo per unit of basis weight expressed as grams per square meter, or gsm, and can have a good clo:gsm at a number of wash cycles, particularly at the longer number of wash cycles. It is desirable to maintain a good clo value over time and over a number of wash cycles per unit basis weight to allow one the flexibility of lowering the amount of fiber fill while maintaining a target clo value or, at a higher target fiber fill, increasing and maintaining higher clo values. The fiber blend, or the nonwoven web (including battings) can have a clo:gsm value at 10 wash cycles of at least 0.014 clo/gsm, or at least 0.015 clo/gsm, or at least 0.016 clo/gsm; or can have a clo:gsm value at 20 wash cycles of at least 0.012 clo/gsm, or at least 0.013 clo/gsm. Thus, there is provided a fiber fill, non-woven web, batting, interliner, or any other articles mentioned that has good thermal insulation after multiple wash cycles even without the necessity of exceeding the basis weight levels of commercially available outerwear, yet contain sustainable and optionally biodegradable fibers.

In one embodiment or in combination with any mentioned embodiments, the fiber blend, or the nonwoven web, can maintain good clo values with minimal loss of clo over wash cycles after initial washing. For example, the fiber blend, or the nonwoven web (including battings) can have a loss of clo value between 5 and 20 wash cycles of not more than 0.015 clo units, or not more than 0.013 clo units.

In one embodiment or in combination with any mentioned embodiments, the fiber blend, or the nonwoven web, can exhibit a short-term compression recovery that is equal to, or exceeding, the short-term compressive recovery of a Comparative Blend, as determined according the ASTM D6571-01 Standard Test Method for Determination of Compression Resistance and Recovery Properties of Highloft Nonwoven Fabric Using Static Force Loading method.

For example, a short-term compressive recovery of a fiber blend or batting made with a combination of CA staple fibers having a dpf of 3.0 or less and staple fibers having a dpf of 6.0 or more is equal to and even higher than the short-term compressive recovery of fiber battings made with 100% of the individual staple fibers. One would expect that, if structural fibers provide the basis for compressive recovery, a reduction in the amount of the structural fiber by blending CA staple fibers having a dpf of 3.0 or less would have the effect of reducing the compressive recovery, particularly when 100% of the staple fibers having a dpf of 3.0 or less have the least compressive recovery. However, we have observed that a surprising enhancement of compressive recovery can be achieve with blends of the staple fibers as described herein, even across a wide variety of blended quantities. In one embodiment or in any of the mentioned embodiments, the short-term compression recovery of the fiber blend, batting, or non-woven article is higher than either of the individual fibers used at 100% (excluding binder fibers), optionally by at least 1%, or at least 2%, or at least 3%, or at least 4%.

In one embodiment, the dpf of the CA fibers of a fiber blend, batting, or non-woven article having a short-term compression recovery that is higher than either of the individual fibers used at 100% (excluding binder fibers), is 2.2 or less, or 2.0 or less, or 1.9 or less.

The nonwoven web may also exhibit desirable levels of softness and/or opacity. Softness is measured according to the Emtec Tissue Softness Analyzer (TSA) method as described in the Example Section below. In some embodiments, the hand-feel of the nonwoven web can be at least 104, 104.5, 105, 105.5, 106, 106.25, 106.5, 106.75, 107, 107.25, 107.5, 107.75, or 108, as determined by the TSA method using the QA1 algorithm. Additionally, or in the alternative, the real softness of the nonwoven web, measured according to the TSA method, can be at least 2, 2.05, 2.10, 2.15, 2.20, 2.25, 2.30, 2.35, 2.40, 2.45, 2.50, 2.55, 2.60, 2.65, 2.70, 2.75, 2.80, 2.85, 2.90, 2.95, 3, 3.05, 3.1, 3.15, 3.2, 3.25, 3.3, 3.35, or 3.4 dB and/or not more than 6, 5.75, 5.5, 5.25, 5.0, 4.75, 4.50, 4.45, 4.40, 4.35, 4.30, 4.25, 4.20, 4.15, 4.10, 4.05, 4.0, 3.95, 3.90, 3.85, 3.80, 3.75, 3.7, 3.65, 3.6, 3.55, 3.5, or 3.45 dB.

In some embodiments, the roughness of the nonwoven web can be at least 1, 2, 5, 8, 10, 12, 12.5, 13, 13.5, 14, 14.5, 15, 15.5, 16, 16.5, 17, 17.5, 18, 18.5, or 19 dB and/or not more than 30, 28, 25, 24, 22.5, 22, 21.5, 21, 20.5, 20, 19.5, 19, 18.5, 18, 17.5, 17, 16.5, 16, 15.5, 15, 14.5, or 14 dB. The web roughness measured according to the TSA method correlates to the vertical vibration of the tissue sample itself caused by the horizontal motion of the blade and the surface structure.

The opacity of a nonwoven web may be measured according to the procedure described in NWSP 060.1.R0. The nonwoven web may have an opacity of at least 40, 45, 50, 55, 60, 65, 70, 75, 80, 85, 90, 95, or up to 100 percent. Alternatively, or in addition, the nonwoven web may have an opacity of not more than 95, 90, 85, 80, 75, 70, 65, 60, or 55 percent, measured according to the above procedure.

The CA staple fibers or non-woven webs or battings formed therefrom can be biodegradable, meaning that such fibers are expected to decompose under certain environmental conditions. The degree of degradation can be characterized by the weight loss of a sample over a given period of exposure to certain environmental conditions. In some cases, the material used to form the staple fibers, the nonwoven webs, or articles produced from the fibers can exhibit a weight loss of at least 5, 10, 15, or 20 percent after burial in soil for 60 days and/or a weight loss of at least 15, 20, 25, 30, or 35 percent after 15 days of exposure to a typical municipal composter. However, the rate of degradation may vary depending on the particular end use of the fibers, as well as the composition of the remaining article, and the specific test. Exemplary test conditions are provided in U.S. Patent Nos. 5,970,988 and 6,571,802.

In some embodiments, the CA fibers or non-woven webs or battings may be biodegradable and such fibers may be used to form nonwoven webs. The CA fibers or non-woven webs or battings can exhibit enhanced levels of environmental non-persistence, characterized by better-than-expected degradation under various environmental conditions. The fibers and fibrous articles described herein may meet or exceed passing standards set by international test methods and authorities for industrial compostability, home compostability, and/or soil biodegradability.

To be considered "compostable," a material must meet the following four criteria: (1) the material must be biodegradable; (2) the material must be disintegrable; (3) the material must not contain more than a maximum amount of heavy metals; and (4) the material must not be ecotoxic. As used herein, the term "biodegradable" generally refers to the tendency of a material to chemically decompose under certain environmental conditions. Biodegradability can exhibit different degrees of biodegradability, depending on the specific conditions to which it is exposed, the material composition and its form. The term "disintegrable" refers to the tendency of a material to physically decompose into smaller fragments when exposed to certain conditions. Disintegration depends both on the material itself, as well as the physical size and configuration of the article being tested. Ecotoxicity measures the impact of the material on plant life, and the heavy metal content of the material is determined according to the procedures laid out in the standard test method.

The CA staple fibers or non-woven webs or battings can exhibit a biodegradation of at least 70 percent in a period of not more than 50 days, when tested under aerobic composting conditions at ambient temperature (28°C ± 2°C) according to ISO 14855-1 (2012). In some cases, the CA fibers can exhibit a biodegradation of at least 70 percent in a period of not more than 49, 48, 47, 46, 45, 44, 43, 42, 41, 40, 39, 38, or 37 days when tested under these conditions, also called "home composting conditions." These conditions may not be aqueous or anaerobic. In some cases, the CA staple fibers can exhibit a total biodegradation of at least 71, 72, 73, 74, 75, 76, 77, 78, 79, 80, 81, 82, 83, 84, 85, 86, 87, or 88 percent, when tested under according to ISO 14855-1 (2012) for a period of 50 days under home composting conditions. This may represent a relative biodegradation of at least 95, 97, 99, 100, 101, 102, or 103 percent, when compared to cellulose subjected to identical test conditions.

To be considered "biodegradable," under home composting conditions according to the French norm NF T 51-800 and the Australian standard AS 5810, a material must exhibit a biodegradation of at least 90 percent in total (e.g., as compared to the initial sample), or a biodegradation of at least 90 percent of the maximum degradation of a suitable reference material after a plateau has been reached for both the reference and test item. The maximum test duration for biodegradation under home compositing conditions is 1 year. The CA staple fibers or non-woven webs or battings may exhibit a biodegradation of at least 90 percent within not more than 1 year, measured according 14855-1 (2012) under home composting conditions. In some cases, the CA staple fibers may exhibit a biodegradation of at least 91, 92, 93, 94, 95, 96, 97, 98, 99, or 99.5 percent within not more than 1 year, or the fibers may exhibit 100 percent biodegradation within not more than 1 year, measured according 14855-1 (2012) under home composting conditions.

Additionally, or in the alternative, the CA fibers or non-woven webs or battings may exhibit a biodegradation of at least 90 percent within not more than 350, 325, 300, 275, 250, 225, 220, 210, 200, 190, 180, 170, 160, 150, 140, 130, 120, 110, 100, 90, 80, 70, 60, or 50 days, measured according 14855-1 (2012) under home composting conditions. In some cases, the fibers can be at least 97, 98, 99, or 99.5 percent biodegradable within not more than 70, 65, 60, or 50 days of testing according to ISO 14855-1 (2012) under home composting conditions. As a result, the CA fibers or non-woven webs or battings may be considered biodegradable according to, for example, French Standard NF T 51-800 and Australian Standard AS 5810 when tested under home composting conditions.

The CA fibers or non-woven webs or battings can exhibit a biodegradation of at least 60 percent in a period of not more than 45 days, when tested under aerobic composting conditions at a temperature of 58°C (± 2°C) according to ISO 14855-1 (2012). In some cases, the fibers can exhibit a biodegradation of at least 60 percent in a period of not more than 44, 43, 42, 41, 40, 39, 38, 37, 36, 35, 34, 33, 32, 31, 30, 29, 28, or 27 days when tested under these conditions, also called "industrial composting conditions." These may not be aqueous or anaerobic conditions. In some cases, the fibers or non-woven webs or battings can exhibit a total biodegradation of at least 65, 70, 75, 80, 85, 87, 88, 89, 90, 91, 92, 93, 94, or 95 percent, when tested under according to ISO 14855-1 (2012) for a period of 45 days under industrial composting conditions. This may represent a relative biodegradation of at least 95, 97, 99, 100, 102, 105, 107, 110, 112, 115, 117, or 119 percent, when compared to cellulose fibers subjected to identical test conditions.

To be considered "biodegradable," under industrial composting conditions according to ASTM D6400 and ISO 17088, at least 90 percent of the organic carbon in the whole item (or for each constituent present in an amount of more than 1% by dry mass) must be converted to carbon dioxide by the end of the test period when compared to the control or in absolute. According to European standard ED 13432 (2000), a material must exhibit a biodegradation of at least 90 percent in total, or a biodegradation of at least 90 percent of the maximum degradation of a suitable reference material after a plateau has been reached for both the reference and test item. The maximum test duration for biodegradability under industrial compositing conditions is 180 days. The CA fibers or non-woven webs or battings described herein may exhibit a biodegradation of at least 90 percent within not more than 180 days, measured according 14855-1 (2012) under industrial composting conditions. In some cases, the CA fibers or non-woven webs or battings may exhibit a biodegradation of at least 91, 92, 93, 94, 95, 96, 97, 98, 99, or 99.5 percent within not more than 180 days, or the fibers may exhibit 100 percent biodegradation within not more than 180 days, measured according 14855-1 (2012) under industrial composting conditions.

Additionally, or in the alternative, the CA fibers or non-woven webs or battings may exhibit a biodegradation of least 90 percent within not more than 175, 170, 165, 160, 155, 150, 145, 140, 135, 130, 125, 120, 115, 110, 105, 100, 95, 90, 85, 80, 75, 70, 65, 60, 55, 50, or 45 days, measured according 14855-1 (2012) under industrial composting conditions. In some cases, the CA fibers or non-woven webs or battings can be at least 97, 98, 99, or 99.5 percent biodegradable within not more than 65, 60, 55, 50, or 45 days of testing according to ISO 14855-1 (2012) under industrial composting conditions. As a result, the CA fibers or non-woven webs or battings may be considered biodegradable according ASTM D6400 and ISO 17088 when tested under industrial composting conditions.

The fibers or non-woven webs or battings may exhibit a biodegradation in soil of at least 60 percent within not more than 130 days, measured according to ISO 17556 (2012) under aerobic conditions at ambient temperature. In some cases, the fibers can exhibit a biodegradation of at least 60 percent in a period of not more than 130, 120, 110, 100, 90, 80, or 75 days when tested under these conditions, also called "soil composting conditions." These may not be aqueous or anaerobic conditions. In some cases, the fibers can exhibit a total biodegradation of at least 65, 70, 72, 75, 77, 80, 82, or 85 percent, when tested under according to ISO 17556 (2012) for a period of 195 days under soil composting conditions. This may represent a relative biodegradation of at least 70, 75, 80, 85, 90, or 95 percent, when compared to cellulose fibers subjected to identical test conditions.

In order to be considered "biodegradable," under soil composting conditions according the OK biodegradable SOIL conformity mark of Vingotte and the DIN Geprüft Biodegradable in soil certification scheme of DIN CERTCO, a material must exhibit a biodegradation of at least 90 percent in total (e.g., as compared to the initial sample), or a biodegradation of at least 90 percent of the maximum degradation of a suitable reference material after a plateau has been reached for both the reference and test item. The maximum test duration for biodegradability under soil compositing conditions is 2 years. The CA fibers or non-woven webs or battings may exhibit a biodegradation of at least 90 percent within not more than 2 years, 1.75 years, 1 year, 9 months, or 6 months measured according ISO 17556 (2012) under soil composting conditions. In some cases, the CA fibers may exhibit a biodegradation of at least 91, 92, 93, 94, 95, 96, 97, 98, 99, or 99.5 percent within not more than 2 years, or the fibers may exhibit 100 percent biodegradation within not more than 2 years, measured according ISO 17556 (2012) under soil composting conditions.

Additionally, or in the alternative, the CA fibers or non-woven webs or battings may exhibit a biodegradation of at least 90 percent within not more than 700, 650, 600, 550, 500, 450, 400, 350, 300, 275, 250, 240, 230, 220, 210, 200, or 195 days, measured according 17556 (2012) under soil composting conditions. In some cases, the CA fibers or non-woven webs or battings can be at least 97, 98, 99, or 99.5 percent biodegradable within not more than 225, 220, 215, 210, 205, 200, or 195 days of testing according to ISO 17556 (2012) under soil composting conditions. As a result, the CA fibers may meet the requirements to receive the OK biodegradable SOIL conformity mark of Vingotte and to meet the standards of the DIN Geprüft Biodegradable in soil certification scheme of DIN CERTCO.

In some embodiments, the CA fibers or non-woven webs or battings may include less than 1, 0.75, 0.50, or 0.25 weight percent of components of unknown biodegradability. In some cases, the fibers or non-woven webs or battings described herein may include no components of unknown biodegradability.

In addition to being biodegradable under industrial and/or home composting conditions, the CA fibers or non-woven webs or battings as described herein may also be compostable under home and/or industrial conditions. As described previously, a material is considered compostable if it meets or exceeds the requirements set forth in EN 13432 for biodegradability, ability to disintegrate, heavy metal content, and ecotoxicity. The CA fibers or non-woven webs or battings may exhibit sufficient compostability under home and/or industrial composting conditions to meet the requirements to receive the OK compost and OK compost HOME conformity marks from Vingotte.

In some cases, the CA fibers or non-woven webs or battings may have a volatile solids concentration, heavy metals and fluorine content that fulfill all of the requirements laid out by EN 13432 (2000). Additionally, the CA fibers or non-woven webs or battings may not cause a negative effect on compost quality (including chemical parameters and ecotoxicity tests).

In some cases, the CA fibers or non-woven webs or battings can exhibit a disintegration of at least 90 percent within not more than 26 weeks, measured according to ISO 16929 (2013) under industrial composting conditions. In some cases, the fibers or non-woven webs or battings may exhibit a disintegration of at least 91, 92, 93, 94, 95, 96, 97, 98, 99, or 99.5 percent under industrial composting conditions within not more than 26 weeks, or the fibers or articles may be 100 percent disintegrated under industrial composting conditions within not more than 26 weeks. Alternatively, or in addition, the fibers or non-woven webs or battings may exhibit a disintegration of at least 90 percent under industrial compositing conditions within not more than 26, 25, 24, 23, 22, 21, 20, 19, 18, 17, 16, 15, 14, 13, 12, 11, or 10 weeks, measured according to ISO 16929 (2013). In some cases, the CA fibers or non-woven webs or battings may be at least 97, 98, 99, or 99.5 percent disintegrated within not more than 12, 11, 10, 9, or 8 weeks under industrial composting conditions, measured according to ISO 16929 (2013).

In some cases, the CA fibers or non-woven webs or battings can exhibit a disintegration of at least 90 percent within not more than 26 weeks, measured according to ISO 16929 (2013) under home composting conditions. In some cases, the fibers or non-woven webs or battings may exhibit a disintegration of at least 91, 92, 93, 94, 95, 96, 97, 98, 99, or 99.5 percent under home composting conditions within not more than 26 weeks, or the fibers or articles may be 100 percent disintegrated under home composting conditions within not more than 26 weeks. Alternatively, or in addition, the fibers or non-woven webs or battings may exhibit a disintegration of at least 90 percent within not more than 26, 25, 24, 23, 22, 21, 20, 19, 18, 17, 16, or 15 weeks under home composting conditions, measured according to ISO 16929 (2013). In some cases, the CA fibers or non-woven webs or battings may be at least 97, 98, 99, or 99.5 percent disintegrated within not more than 20, 19, 18, 17, 16, 15, 14, 13, or 12 weeks, measured under home composting conditions according to ISO 16929 (2013).

The nonwoven web, optionally thermally bonded, made with the CA fibers is particularly suited for use as a heat-insulating interliner or layer in textile-type applications, such as in garment, bedding, and other household goods. In such applications, the heat-insulating interliner may be used by itself or in combination with other insulating materials, such as down, feather, polyester fibers, polyester microfibers, or mixtures thereof. Examples of articles of manufacturer that can include the heat-insulating interliner include outerwear, shoes, gloves, pillows, comforters, blankets, throws, mattresses, mattress pads, sleeping bags, cushions, and the like.

In some cases, the nonwoven web can have superior heat-insulating properties for its weight. For example, the web can have a clo per gsm (or clo/(g/m²)) value of at least 0.020, or at least 0.022, or at least 0.024, or at least 0.026 g/m², and/or up to 0.30, or up to 0.28, or up to 0.27 g/m².

To remove any doubt, the present invention includes and expressly contemplates and discloses any and all combinations of embodiments, features, characteristics, parameters, and/or ranges mentioned herein. That is, the subject matter of the present invention may be defined by any combination of embodiments, features, characteristics, parameters, and/or ranges mentioned herein.

It is contemplated that any ingredient, component, or step that is not specifically named or identified as part of the present invention may be explicitly excluded.

Any process/method, apparatus, compound, composition, embodiment, or component of the present invention may be modified by the transitional terms "comprising," "consisting essentially of," or "consisting of," or variations of those terms.

As used herein, the indefinite articles "a" and "an" mean one or more, unless the context clearly suggests otherwise. Similarly, the singular form of nouns includes their plural form, and vice versa, unless the context clearly suggests otherwise.

While attempts have been made to be precise, the numerical values and ranges described herein should be considered as approximations, unless the context indicates otherwise. These values and ranges may vary from their stated numbers depending upon the desired properties sought to be obtained by the present disclosure as well as the variations resulting from the standard deviation found in the measuring techniques. Moreover, the ranges described herein are intended and specifically contemplated to include all sub-ranges and values within the stated ranges. For example, a range of 50 to 100 is intended to include all values within the range including sub-ranges such as 60 to 90, 70 to 80, etc.

Any two numbers of the same property or parameter reported in the working examples may define a range. Those numbers may be rounded off to the nearest thousandth, hundredth, tenth, whole number, ten, hundred, or thousand to define the range.

The content of all documents cited herein, including patents, patent applications, as well as non-patent literature, is hereby incorporated by reference in their entirety. To the extent that any incorporated subject matter contradicts with any disclosure herein, the disclosure herein shall take precedence over the incorporated content.

This invention can be further illustrated by the following working examples, although it should be understood that these examples are included merely for purposes of illustration and are not intended to limit the scope of the invention.

### EXAMPLES

### Examples 1-5: Preparation of Thermally-Bonded, Nonwoven Battings (Examples 3 and 5 are not according to the present invention)

The fiber blends listed in Table 1 below were converted into high-loft nonwoven battings using a commercial carding and cross-lapping line. The target weight for each batting was 100 g/m². Table 1 sets forth a summary of the composition of each example.

**Table 1: Compositions**

| **Example No.** | **Cellulose Acetate Base Fiber(s) (wt. %, dpf, cross-sectional shape)** | **Structural Fiber (wt. %)** | **Binder Fiber (wt. %)** | **Comments** |
|---|---|---|---|---|
| 1 | 55% 1.8Y | 25% | 20% | |
| 2 | 55% 1.8R | 25% | 20% | |
| 3 | 30% 1.8Y | 50% | 20% | |
| 4 | 55% 1.8Y | 25% | 20% | Vacuum packed |
| 5 | 30% 1.8Y | 50% | 20% | Vacuum packed |

The weight percentage in Table 1 are based on the entire batting. The 3.0 dpf or less fibers used were:
1.8 dpf with a trilobal (Y) cross-section, 17 crimps per inch, 51 mm cut length
1.8 dpf with a round (R) cross-section, 17 crimps per inch, 38 mm cut length

The structural staple fiber used was:
7 dpf conjugated (three dimensional crimp) hollow polyester staple fiber with 51 mm cut length

The binder staple fiber used was:
3 dpf polyester/copolyester (core/sheath) bicomponent with 51 mm cut length

The Reference examples are commercially available blends used in outerwear to determine the range of acceptable clo and loft:
Sample A - A commercially available insulated jacket with polyester face and liner fabric and a 60 g/m² insulation layer with scrim Sample B - A commercially available insulated jacket with polyester face and liner fabric and an 80 g/m² insulation layer Sample C - A commercially available insulated jacket with polyester face and liner fabric and a 100 g/m² insulation layer Sample D - A commercially available insulated jacket with cotton/polyester face fabric and nylon liner fabric and an 80 g/m² insulation layer with scrim.

For all examples with CA fiber, the bales were opened and the fiber was weighed and blended before being fed into the card. After exiting the card, the web was cross-lapped and passed through an oven at around 185°C for thermal bonding. The edges of the batting were trimmed off and the batting was collected on rolls. Compressed versions of examples 1 and 2 (samples 4 and 5 in Table 1) were also collected by placing the rolls in a vacuum bag and removing the air. These compressed versions remained in their vacuum bag for 3 months before the bags were opened and the battings were allowed to recover to their high-loft state.

### Construction of Garment Mock-Ups

Garment mock-ups were created by sewing the insulation battings between face and liner fabrics. The face and liner fabric was a 100% polyester ripstop with an air permeability of 2.97 ft³/(ft²/min) (1 ft³ = 28.3168 liters, 1 ft²/min = 0.092903 m²/min) and a weight of 27.6 g/m². The garment mock-ups were 12 inches by 12 inches (1 inch = 2.54 cm) in size and a quilt line was placed every 4 inches to secure the insulation to the face fabric. The liner was free hanging. An illustration of the garment mock-ups is provided in Figure 1.

### Laundry Durability Testing

Laundry durability testing was performed in a Kenmore 400 Series top-load washing machine with a center agitator. The garment mock-ups, comparative examples, and ballast fabric were added to the machine to achieve a total load weight of 4 lbs (1 lb = 0.453592 kg). The washing machine was filled with water using the medium load size setting, which correlates to approximately 18 gallons (1 gallon = 3.78541 liters) on our machine. The warm water setting was used. AATCC standard reference detergent was added and the mock-ups were laundered using the normal cycle. Following the wash cycle, the mock-ups, comparative examples and ballast fabric were tumble dried in a Maytag Centennial dryer using the low temperature setting for 60 minutes.

The data presented under wash cycles represents the total number of wash and dry cycles. For example, data presented at 20 wash cycles was obtained after 20 cycles of washing and drying as opposed to 20 cycles of washing followed by a single cycle of drying. Drying after each wash cycle is more representative of consumer behavior.

### Thermal Resistance Testing

Each sample was tested for initial thermal resistance in accordance with ASTM D1518-14 Standard Test Method for Thermal Resistance of Batting Systems Using a Hot Plate using Option 2: Air Velocity Condition. The chamber temperature was set at 15ºC. The relative humidity was controlled to 70%. The air velocity was 1.0 m/second. The average total thermal resistance was recorded and used to calculate intrinsic Clo.

Subsequently, each sample was laundered for 20 wash and dry cycles. At cycles 1, 3, 5, 10 and 20, the samples were tested for thermal resistance according to the procedure noted above. The results are reported in Table 2 below.

**Table 2: Clo At Wash Cycles**

| **Example No.** | **Initial Clo** | **Clo at 1 wash cycle** | **Clo at 3 wash cycles** | **Clo at 5 wash cycles** | **Clo at 10 wash cycles** | **Clo at 20 wash cycles** |
|---|---|---|---|---|---|---|
| 1 | 2.549 | 1.711 | 1.451 | 1.433 | 1.377 | 1.249 |
| 2 | 2.306 | 1.602 | 1.307 | 1.341 | 1.305 | 1.012 |
| 3 | 2.663 | 1.970 | 1.700 | 1.765 | 1.686 | 1.534 |
| 4 | 2.202 | 1.448 | 1.405 | 1.344 | 1.213 | 1.252 |
| 5 | 2.067 | 1.648 | 1.613 | 1.600 | 1.517 | 1.433 |
| Reference Sample A | 1.328 | 1.303 | 1.189 | 1.253 | 1.242 | 1.112 |
| Reference Sample B | 1.287 | 1.417 | 1.219 | 1.263 | 1.175 | 1.089 |
| Reference Sample C | 1.869 | 2.086 | 1.869 | 1.912 | 1.754 | 1.551 |
| Reference Sample D | 1.590 | 1.442 | 1.413 | 1.445 | 1.362 | 1.249 |

As seen from Table 2, battings containing CA fiber have higher initial clo values than any of the commercially available comparative samples. After the first, third, fifth, tenth, and 20^{th} laundering cycles, battings containing CA fiber can be made within the window of commercially acceptable clo values as shown by the commercially available Reference samples.

The clo values per unit basis weight were also determined and reported below in Table 3. Even at or after the fifth, tenth, and 20^{th} laundering cycles, battings containing CA fiber can be made within the window of commercially acceptable clo values per unit basis weight as shown by the commercially available Reference samples.

**Table 3**

| **Example No.** | **Initial Clo** | **Clo at 1 wash cycle** | **Clo at 3 wash cycles** | **Clo at 5 wash cycles** | **Clo at 10 wash cycles** | **Clo at 20 wash cycles** |
|---|---|---|---|---|---|---|
| Reference Sample A | 0.022 | 0.022 | 0.020 | 0.021 | 0.021 | 0.019 |
| Reference Sample B | 0.016 | 0.018 | 0.015 | 0.016 | 0.015 | 0.014 |
| Reference Sample C | 0.019 | 0.021 | 0.019 | 0.019 | 0.018 | 0.016 |
| Reference Sample D | 0.020 | 0.018 | 0.018 | 0.018 | 0.017 | 0.016 |
| **1** | 0.025 | 0.017 | 0.015 | 0.014 | 0.014 | 0.012 |
| **2** | 0.023 | 0.016 | 0.013 | 0.013 | 0.013 | 0.010 |
| **3** | 0.027 | 0.020 | 0.017 | 0.018 | 0.017 | 0.015 |
| **4** | 0.022 | 0.014 | 0.014 | 0.013 | 0.012 | 0.013 |
| **5** | 0.021 | 0.016 | 0.016 | 0.016 | 0.015 | 0.014 |

### Loft Testing

The loft of each sample was tested at the same intervals that thermal resistance was tested; e.g. initial and at 1, 3, 5, 10, and 20 wash cycles. The results are reported below in Table 4.

**Table 4: Loft After Laundering**

| **Example No.** | **Initial Loft (mm)** | **Loft at 1 wash cycle (mm)** | **Loft at 3 wash cycles (mm)** | **Loft at 5 wash cycles (mm)** | **Loft at 10 wash cycles (mm)** | **Loft at 20 wash cycles (mm)** |
|---|---|---|---|---|---|---|
| 1 | 19.10 | 10.71 | 9.28 | 8.84 | 7.94 | 6.86 |
| 2 | 16.46 | 9.22 | 8.16 | 7.54 | 7.12 | 5.68 |
| 3 | 18.25 | 13.04 | 12.19 | 10.82 | 11.06 | 9.12 |
| 4 | 16.57 | 10.00 | 7.87 | 6.65 | 7.08 | 6.50 |
| 5 | 13.90 | 12.44 | 9.28 | 8.76 | 7.79 | 8.07 |
| Reference Sample A | 7.41 | 7.58 | 7.62 | 6.65 | 7.13 | 6.37 |
| Reference Sample B | 8.12 | 8.34 | 7.40 | 8.14 | 7.14 | 6.56 |
| Reference Sample C | 10.91 | 13.70 | 11.70 | 11.50 | 11.05 | 9.86 |
| Reference Sample D | 10.09 | 9.20 | 8.88 | 8.47 | 8.20 | 8.34 |

As seen from Table 4, battings containing CA fiber have higher initial lofts than any of the commercially available comparative samples. After the first, third, fifth, tenth, and 20^{th} laundering cycles, battings containing CA fibers can be made within the window of commercially acceptable lofts as shown by the commercially available Reference samples.

The results tabulated in Tables 2, 3, and 4 are depicted visually in Figures 2, 3, and 4, respectively to further illustrate that sustainable CA fibers can replace a portion of petroleum-based staple fibers while obtaining comparable, or in some instances, better thermal insulation values, having good clo values after multiple wash cycles per unit basis weight, and further, maintain or in some instances improve the loft. The CA fibers used can also be biodegradable, thus providing a sustainable, biodegradable high performing fiber fill, non-woven web, interliner, or articles made therefrom.

### Examples 6-14: Preparation of Nonwoven Battings

The fiber blends listed in Table 5 were converted into high-loft nonwoven battings using a Ramella carding machine. All examples were produced at equivalent basis weights. Table 5 sets forth a summary of the composition of each example. These examples are not according to the present invention.

**Table 5: Compositions**

| **Example No.** | **1.8Y (wt. %)** | **3.0Y (wt. %)** | **8.0Y (wt. %)** |
|---|---|---|---|
| 6 | 100% | | |
| 7 | | 100% | |
| 8 | | | 100% |
| 9 | 25% | | 75% |
| 10 | 50% | | 50% |
| 11 | 75% | | 25% |
| 12 | | 25% | 75% |
| 13 | | 50% | 50% |
| 14 | | 75% | 25% |

The CA fibers used were:
1.8 dpf with a trilobal (Y) cross-section, 14 crimps per inch, 51 mm cut length
3.0 dpf with a trilobal (Y) cross-section, 17 crimps per inch, 51 mm cut length
8.0 dpf with a trilobal (Y) cross-section, 17 crimps per inch, 51 mm cut length

For each example, the necessary fibers were weighed to attain the correct blend ratio and mixed by hand prior to being fed into the card. Upon exiting the card, the resulting web was collected on a rotating drum. The web was allowed to overlap as the drum rotated to produce the high-loft nonwoven batting. Once all of the fiber had run through the card, the overlapped batting was removed from the drum and stored in a flat state with nothing on top of it to compress it. This process was repeated until all of the aforementioned examples were created.

### Compression Resistance and Recovery Testing

Examples 6-14 were tested for compression resistance and recovery according to ASTM D6571-01 Standard Test Method for Determination of Compression Resistance and Recovery Properties of Highloft Nonwoven Fabric Using Static Force Loading. The results are reported in Table 6.

**Table 6: Compression Resistance and Recovery**

| **Example No.** | **Average Initial Loft (mm)** | **Average 10-Minute Compressed Loft (mm)** | **Compression Resistance (%)** | **Average 10-Minute Relaxed Loft (mm)** | **Average 1-Hour Recovery Loft (mm)** | **Short-Term Compression Recovery (%)** |
|---|---|---|---|---|---|---|
| 6 | 95.25 | 19.50 | **20.47** | 60.25 | 37.25 | **61.83** |
| 7 | 85.00 | 22.00 | **25.88** | 64.50 | 44.25 | **68.60** |
| 8 | 89.50 | 25.50 | **28.49** | 68.00 | 43.75 | **64.34** |
| 9 | 86.00 | 23.00 | **26.74** | 61.25 | 41.75 | **68.16** |
| 10 | 94.25 | 22.25 | **23.61** | 66.50 | 46.75 | **70.30** |
| 11 | 83.50 | 18.50 | **22.16** | 57.00 | 38.00 | **66.67** |
| 12 | 85.75 | 23.00 | **26.82** | 62.25 | 42.25 | **67.87** |
| 13 | 87.25 | 22.75 | **26.07** | 64.75 | 42.75 | **66.02** |
| 14 | 87.75 | 22.25 | **25.36** | 62.75 | 43.00 | **68.53** |

As seen from Table 6, the compression resistance of the battings containing only one fiber type shows that sample 8 at 8.0Y provides to most compression resistance, followed by sample 7 at 3.0Y, and then sample 6 at 1.8Y. In blends of 1.8Y and 8.0Y, a higher fraction of 8.0Y gives more compression resistance. The same is true for blends of 3.0Y and 8.0Y. Blends of 3.0Y and 8.0Y provide greater compression resistance than blends of 1.8Y and 8.0Y produced at the same blend ratio (*i.e.,* example 12 has greater compression resistance than example 9, example 13 has greater compression resistance than example 10, and example 14 has greater compression resistance than example 11).

Table 6 also provides short-term recovery data following 24 hours of compression and one hour of recovery. Of the battings containing only one fiber type, 3.0Y gives the greatest short-term recovery, followed by 8.0Y, and then 1.8Y. Surprisingly, blends of 1.8Y and 8.0Y give greater short-term recovery than 1.8Y or 8.0Y alone. This synergistic effect is most significant for example 10 (50% 1.8Y + 50% 8.0Y), which gives the greatest short-term recovery of the data set.

The results tabulated in 6 are depicted in Figures 5 and 6, respectively to further illustrate that higher denier CA fibers can be incorporated into highloft nonwoven battings to improve compression resistance and recovery.

The invention has been described in detail with particular reference to specific embodiments thereof, but it will be understood that variations and modifications can be made within the scope of the invention.

## Claims

1. A fiber blend comprising:
(a) cellulose acetate (CA) staple fibers having a denier per filament (DPF) of 3.0 or less, in an amount ranging from 45 to 60 wt% based on the total weight of the fiber blend;
(b) structural staple fibers having a dpf of 6.0 or more, in an amount ranging from 20 to 35 wt% based on the total weight of the fiber blend; and
(c) binder fibers, in an amount ranging from 0 to 30 wt% based on the total weight of the fiber blend.

2. The blend of claim 1, wherein the CA staple fibers have a DPF of not more than 2.0.

3. The blend of claim 1 or 2, wherein the CA staple fibers have or are obtained from filaments that have a crimp frequency of 8 to 25 crimps per inch (CPI), are Y- or round-shaped, and have a cut length of 10 to 55 mm.

4. The blend of any one of claims 1 to 3, comprising at least two different CA staple fibers, each having a DPF of not more than 3.0, wherein the difference between the at least two different CA fibers is one or more of:
a. DPF,
b. CPI, or
c. shape.

5. The blend of any one of claims 1 to 4, wherein the structural staple fibers comprise CA staple fibers.

6. A nonwoven web, batting, fiber fill, or interliner comprising the blend of any one of claims 1 to 5.

7. The nonwoven web, batting, fiber fill, or interliner of claim 6, comprising a nonwoven web or batting having an initial clo:mm value of at least 0.210.

8. The nonwoven web, batting, fiber fill, or interliner of claim 6 or 7, comprising a non-woven web or batting having a short-term compression recovery that is equal to, or exceeding, the short-term compression recovery of a web or batting replacing the blend of said fibers with 100% of either of the staple fibers having a dpf of 3.0 or less or said structural fibers ("Comparative Blend"), as determined according the ASTM D6571-01 Standard Test Method for Determination of Compression Resistance and Recovery Properties of Highloft Nonwoven Fabric Using Static Force Loading method; preferably the nonwoven web, batting, fiber fill, or interliner of claim 6 or 7, comprising a non-woven web or batting having a short-term compression recovery that is 2% higher than the short-term compression recovery of the Comparative Blend.

9. The nonwoven web, batting, fiber fill, or interliner of any one of claims 6 to 8, comprising a non-woven web or batting wherein the article comprises a garment, a shoe, a glove, a pillow, a comforter, a blanket, a throw, a mattress, a mattress pad, a sleeping bag, or a cushion.

10. The nonwoven web, batting, fiber fill, or interliner of claim 6, comprising a nonwoven web that is air-laid.

11. A bale comprising the fiber blend of any one of claims 1 to 5.

## Patentansprüche

1. Fasermischung, umfassend:
(a) Celluloseacetat(CA)-Stapelfasern, die ein Denier pro Filament (DPF) von 3,0 oder weniger aufweisen, in einer Menge von 45 bis 60 Gew.-%, basierend auf dem Gesamtgewicht der Fasermischung;
(b) Strukturstapelfasern, die ein dpf von 6,0 oder mehr aufweisen, in einer Menge von 20 bis 35 Gew.-%, basierend auf dem Gesamtgewicht der Fasermischung; und
(c) Bindefasern in einer Menge von 0 bis 30 Gew.-%, basierend auf dem Gesamtgewicht der Fasermischung.

2. Mischung nach Anspruch 1, wobei die CA-Stapelfasern ein DPF von nicht mehr als 2,0 aufweisen.

3. Mischung nach Anspruch 1 oder 2, wobei die CA-Stapelfasern Filamente, die eine Kräuselfrequenz von 8 bis 25 Kräuselungen pro Zoll (CPI) aufweisen, aufweisen oder daraus erhalten sind, Y- oder rundförmig sind und eine Schnittlänge von 10 bis 55 mm aufweisen.

4. Mischung nach einem der Ansprüche 1 bis 3, umfassend mindestens zwei verschiedene CA-Stapelfasern, die jeweils ein DPF von nicht mehr als 3,0 aufweisen, wobei der Unterschied zwischen den mindestens zwei verschiedenen CA-Fasern eines oder mehrere von Folgendem ist:
a. DPF,
b. CPI oder
c. Form.

5. Mischung nach einem der Ansprüche 1 bis 4, wobei die Strukturstapelfasern CA-Stapelfasern umfassen.

6. Vliesstoff, Wattierung, Faserfüllung oder Zwischenlage, umfassend die Mischung nach einem der Ansprüche 1 bis 5.

7. Vliesstoff, Wattierung, Faserfüllung oder Zwischenlage nach Anspruch 6, umfassend einen Vliesstoff oder eine Wattierung, aufweisend einen anfänglichen Clo:mm-Wert von mindestens 0,210.

8. Vliesstoff, Wattierung, Faserfüllung oder Zwischenlage nach Anspruch 6 oder 7, umfassend einen Vliesstoff oder eine Wattierung, aufweisend ein Kurzzeit-Rückstellvermögen, das gleich oder größer ist als das Kurzzeit-Rückstellvermögen eines Stoffs oder einer Wattierung, der/die die Mischung der Fasern durch 100 % entweder der Stapelfasern, die ein dpf von 3,0 oder weniger aufweisen, oder der Strukturfasern ersetzt ("Vergleichsmischung"), bestimmt gemäß dem ASTM D6571-01 Standardtestverfahren zur Bestimmung von Druckfestigkeit und Erholungseigenschaften von Highloft-Vliesstoffen unter Verwendung eines statischen Kraftbelastungsverfahrens; vorzugsweise den Vliesstoff, die Wattierung, die Faserfüllung oder die Zwischenlage nach Anspruch 6 oder 7, umfassend einen Vliesstoff oder eine Wattierung, aufweisend ein Kurzzeit-Rückstellvermögen, das 2 % höher als das Kurzzeit-Rückstellvermögen der Vergleichsmischung ist.

9. Vliesstoff, Wattierung, Faserfüllung oder Zwischenlage nach einem der Ansprüche 6 bis 8, umfassend einen Vliesstoff oder eine Wattierung, wobei der Artikel ein Kleidungsstück, einen Schuh, einen Handschuh, ein Kissen, eine Bettdecke, eine Decke, eine Tagesdecke, eine Matratze, eine Matratzenauflage, einen Schlafsack oder ein Polster umfasst.

10. Vliesstoff, Wattierung, Faserfüllung oder Zwischenlage nach Anspruch 6, umfassend einen luftgelegten Vliesstoff.

11. Bündel, umfassend die Fasermischung nach einem der Ansprüche 1 bis 5.

## Revendications

1. Mélange de fibres comprenant :
(a) des fibres discontinues d'acétate de cellulose (CA) ayant un denier par filament (DPF) inférieur ou égal à 3,0, à une proportion située dans la plage allant de 45 à 60 % en poids par rapport au poids total du mélange de fibres ;
(b) des fibres discontinues structurales ayant un dpf supérieur ou égal à 6,0, à une proportion située dans la plage allant de 20 à 35 % en poids par rapport au poids total du mélange de fibres ; et
(c) des fibres liantes, à une proportion située dans la plage allant de 0 à 30 % en poids par rapport au poids total du mélange de fibres.

2. Mélange selon la revendication 1, dans lequel les fibres discontinues de CA ont un DPF inférieur ou égal à 2,0.

3. Mélange selon la revendication 1 ou 2, dans lequel les fibres discontinues de CA ont ou sont obtenues à partir de filaments qui présentent une fréquence de frisure de 8 à 25 frisures par pouce (CPI), sont rondes ou en forme de Y et ont une longueur de coupe de 10 à 55 mm.

4. Mélange selon l'une quelconque des revendications 1 à 3, comprenant au moins deux fibres discontinues de CA différentes, chacune ayant un DPF inférieur ou égal à 3,0, dans lequel la différence entre les au moins deux fibres de CA différentes porte sur un ou plusieurs des éléments suivants :
a. le DPF,
b. les CPI, ou
c. la forme.

5. Mélange selon l'une quelconque des revendications 1 à 4, dans lequel les fibres discontinues structurales comprennent des fibres discontinues de CA.

6. Bande de non tissé, nappe ouatée, garnissage fibreux ou doublure intercalaire comprenant le mélange selon l'une quelconque des revendications 1 à 5.

7. Bande de non tissé, nappe ouatée, garnissage fibreux ou doublure intercalaire selon la revendication 6, comprenant une bande de non tissé ou une nappe ouatée ayant une valeur initiale d'au moins 0,210 clo:mm.

8. Bande de non tissé, nappe ouatée, garnissage fibreux ou doublure intercalaire selon la revendication 6 ou 7, comprenant une bande de non tissé ou une nappe ouatée ayant une récupération de forme à court terme après compression supérieure ou égale à la récupération de forme à court terme après compression d'une bande ou d'une nappe ouatée remplaçant le mélange desdites fibres par 100 % de l'une quelconque des fibres discontinues ayant un dpf inférieur ou égal à 3,0 ou desdites fibres structurales (« Mélange comparatif »), telle que déterminée selon la méthode d'essai normalisée ASTM D6571-01 pour la détermination de la résistance à la compression et des propriétés de récupération des tissus non tissés à gonflant volumineux par la méthode de chargement de force statique ; de préférence, la bande de non tissé, la nappe ouatée, le garnissage fibreux ou la doublure intercalaire selon la revendication 6 ou 7, comprenant une bande de non tissé ou une nappe ouatée présentant une récupération de forme à court terme après compression supérieure de 2 % à la récupération de forme à court terme après compression du « Mélange comparatif ».

9. Bande de non tissé, nappe ouatée, garnissage fibreux ou doublure intercalaire selon l'une quelconque des revendications 6 à 8, comprenant une bande de non tissé ou une nappe ouatée dans laquelle l'article comprend un vêtement, une chaussure, un gant, un oreiller, une couette, une couverture, un jeté, un matelas, un protège-matelas, un sac de couchage ou un coussin.

10. Bande de non tissé, nappe ouatée, garnissage fibreux ou doublure intercalaire selon la revendication 6, comprenant une bande de non tissé qui est un non-tissé par voie aérodynamique.

11. Balle comprenant le mélange de fibres selon l'une quelconque des revendications 1 à 5.
